



US009139928B2

(12) **United States Patent**  
**Mazyar et al.**

(10) **Patent No.:** **US 9,139,928 B2**  
(b5) **Date of Patent:** **Sep. 22, 2015**

(54) **CORRODIBLE DOWNHOLE ARTICLE AND METHOD OF REMOVING THE ARTICLE FROM DOWNHOLE ENVIRONMENT**

(75) Inventors: **Oleg A. Mazyar**, Houston, TX (US);  
**Matthew T. McCoy**, Richmond, TX (US)

(73) Assignee: **Baker Hughes Incorporated**, Houston, TX (US)

(\*) Notice: Subject to any disclaimer, the term of this patent is extended or adjusted under 35 U.S.C. 154(b) by 585 days.

(21) Appl. No.: **13/162,781**

(22) Filed: **Jun. 17, 2011**

(65) **Prior Publication Data**

US 2012/0318513 A1 Dec. 20, 2012

(51) **Int. Cl.**

**C25D 5/48** (2006.01)  
**C23C 18/16** (2006.01)

(52) **U.S. Cl.**

CPC ..... **C25D 5/48** (2013.01); **C23C 18/1689** (2013.01)

(58) **Field of Classification Search**

None

See application file for complete search history.

(56) **References Cited**

U.S. PATENT DOCUMENTS

|               |         |                             |
|---------------|---------|-----------------------------|
| 1,468,905 A   | 9/1923  | Herman                      |
| 2,238,895 A   | 4/1941  | Gage                        |
| 2,261,292 A   | 11/1941 | Salnikov                    |
| 2,294,648 A   | 9/1942  | Ansel et al.                |
| 2,301,624 A   | 11/1942 | Holt                        |
| 2,754,910 A * | 7/1956  | Derrick et al. .... 166/284 |
| 2,983,634 A   | 5/1961  | Budininkas et al.           |
| 3,057,405 A   | 10/1962 | Mallinger                   |

|             |         |                   |
|-------------|---------|-------------------|
| 3,106,959 A | 10/1963 | Huitt et al.      |
| 3,152,009 A | 10/1964 | DeLong            |
| 3,196,949 A | 7/1965  | Thomas            |
| 3,242,988 A | 3/1966  | McGuire et al.    |
| 3,316,748 A | 5/1967  | Lang et al.       |
| 3,347,317 A | 10/1967 | Zandemer          |
| 3,347,714 A | 10/1967 | Broverman et al.  |
| 3,390,724 A | 7/1968  | Caldwell          |
| 3,395,758 A | 8/1968  | Kelly et al.      |
| 3,406,101 A | 10/1968 | Kilpatrick        |
| 3,434,537 A | 3/1969  | Zandmer           |
| 3,465,181 A | 9/1969  | Colby et al.      |
| 3,513,230 A | 5/1970  | Rhees et al.      |
| 3,637,446 A | 1/1972  | Elliott et al.    |
| 3,645,331 A | 2/1972  | Maurer et al.     |
| 3,765,484 A | 10/1973 | Hamby, Jr. et al. |

(Continued)

FOREIGN PATENT DOCUMENTS

|    |           |         |
|----|-----------|---------|
| CN | 1076968   | 10/1993 |
| CN | 1255879 A | 6/2000  |

(Continued)

OTHER PUBLICATIONS

Notification of Transmittal of the International Search Report and the Written Opinion of the International Searching Authority; PCT/US2010/059257; Korean Intellectual Property Office; Mailed Jul. 27, 2011.

(Continued)

*Primary Examiner* — Doug Hutton, Jr.

*Assistant Examiner* — Anuradha Ahuja

(74) *Attorney, Agent, or Firm* — Cantor Colburn LLP

(57) **ABSTRACT**

A method of removing a corrodible downhole article having a surface coating includes eroding the surface coating by physical abrasion, chemical etching, or a combination of physical abrasion and chemical etching, the surface coating comprising a metallic layer of a metal resistant to corrosion by a corrosive material.

**20 Claims, 2 Drawing Sheets**



| (56)                  | References Cited |                       |               |             |                    |                |  |
|-----------------------|------------------|-----------------------|---------------|-------------|--------------------|----------------|--|
| U.S. PATENT DOCUMENTS |                  |                       |               |             |                    |                |  |
| 3,768,563 A           | 10/1973          | Blount                | 5,061,323 A   | 10/1991     | DeLucia            |                |  |
| 3,775,823 A           | 12/1973          | Adolph et al.         | 5,063,775 A   | 11/1991     | Walker, Sr. et al. |                |  |
| 3,878,889 A           | 4/1975           | Seabourn              | 5,073,207 A   | 12/1991     | Faure et al.       |                |  |
| 3,894,850 A           | 7/1975           | Kovalchuk et al.      | 5,074,361 A   | 12/1991     | Brisco et al.      |                |  |
| 3,924,677 A           | 12/1975          | Prenner et al.        | 5,076,869 A   | 12/1991     | Bourell et al.     |                |  |
| 4,010,583 A           | 3/1977           | Highberg              | 5,084,088 A   | 1/1992      | Okazaki            |                |  |
| 4,039,717 A           | 8/1977           | Titus                 | 5,087,304 A   | 2/1992      | Chang et al.       |                |  |
| 4,050,529 A           | 9/1977           | Tagirov et al.        | 5,090,480 A   | 2/1992      | Pittard et al.     |                |  |
| 4,248,307 A           | 2/1981           | Silberman et al.      | 5,095,988 A   | 3/1992      | Bode               |                |  |
| 4,372,384 A           | 2/1983           | Kinney                | 5,103,911 A   | 4/1992      | Heijnen            |                |  |
| 4,373,584 A           | 2/1983           | Silberman et al.      | 5,117,915 A   | 6/1992      | Mueller et al.     |                |  |
| 4,373,952 A           | 2/1983           | Parent                | 5,161,614 A   | 11/1992     | Wu et al.          |                |  |
| 4,374,543 A           | 2/1983           | Richardson            | 5,178,216 A   | 1/1993      | Giroux et al.      |                |  |
| 4,384,616 A           | 5/1983           | Dellinger             | 5,181,571 A   | 1/1993      | Mueller et al.     |                |  |
| 4,395,440 A           | 7/1983           | Abe et al.            | 5,183,631 A   | 2/1993      | Kugimiya et al.    |                |  |
| 4,399,871 A           | 8/1983           | Adkins et al.         | 5,188,182 A   | 2/1993      | Echols, III et al. |                |  |
| 4,407,368 A *         | 10/1983          | Erbstoesser .....     | 166/284       | 5,188,183 A | 2/1993             | Hopmann et al. |  |
| 4,422,508 A           | 12/1983          | Rutledge, Jr. et al.  | 5,204,055 A   | 4/1993      | Sachs et al.       |                |  |
| 4,452,311 A           | 6/1984           | Speegle et al.        | 5,222,867 A   | 6/1993      | Walker, Sr. et al. |                |  |
| 4,475,729 A           | 10/1984          | Costigan              | 5,226,483 A   | 7/1993      | Williamson, Jr.    |                |  |
| 4,498,543 A           | 2/1985           | Pye et al.            | 5,228,518 A   | 7/1993      | Wilson et al.      |                |  |
| 4,499,048 A           | 2/1985           | Hanejko               | 5,234,055 A   | 8/1993      | Cornette           |                |  |
| 4,499,049 A           | 2/1985           | Hanejko               | 5,253,714 A   | 10/1993     | Davis et al.       |                |  |
| 4,526,840 A           | 7/1985           | Jerabek               | 5,271,468 A   | 12/1993     | Streich et al.     |                |  |
| 4,534,414 A           | 8/1985           | Pringle               | 5,282,509 A   | 2/1994      | Schurr, III        |                |  |
| 4,539,175 A           | 9/1985           | Lichti et al.         | 5,293,940 A   | 3/1994      | Hromas et al.      |                |  |
| 4,554,986 A           | 11/1985          | Jones                 | 5,304,260 A   | 4/1994      | Aikawa et al.      |                |  |
| 4,640,354 A           | 2/1987           | Boisson               | 5,309,874 A   | 5/1994      | Willermet et al.   |                |  |
| 4,664,962 A           | 5/1987           | DesMarais, Jr.        | 5,310,000 A   | 5/1994      | Arterbury et al.   |                |  |
| 4,668,470 A           | 5/1987           | Gilman et al.         | 5,316,598 A   | 5/1994      | Chang et al.       |                |  |
| 4,673,549 A           | 6/1987           | Ecer                  | 5,318,746 A   | 6/1994      | Lashmore           |                |  |
| 4,674,572 A           | 6/1987           | Gallus                | 5,380,473 A   | 1/1995      | Bogue et al.       |                |  |
| 4,678,037 A           | 7/1987           | Smith                 | 5,387,380 A   | 2/1995      | Cima et al.        |                |  |
| 4,681,133 A           | 7/1987           | Weston                | 5,392,860 A   | 2/1995      | Ross               |                |  |
| 4,688,641 A           | 8/1987           | Knieriem              | 5,394,941 A   | 3/1995      | Venditto et al.    |                |  |
| 4,693,863 A           | 9/1987           | Del Corso et al.      | 5,398,754 A   | 3/1995      | Dinhoble           |                |  |
| 4,703,807 A           | 11/1987          | Weston                | 5,407,011 A   | 4/1995      | Layton             |                |  |
| 4,706,753 A           | 11/1987          | Ohkochi et al.        | 5,409,555 A   | 4/1995      | Fujita et al.      |                |  |
| 4,708,202 A           | 11/1987          | Sukup et al.          | 5,411,082 A   | 5/1995      | Kennedy            |                |  |
| 4,708,208 A           | 11/1987          | Halbardier            | 5,417,285 A   | 5/1995      | Van Buskirk et al. |                |  |
| 4,709,761 A           | 12/1987          | Setterberg, Jr.       | 5,427,177 A   | 6/1995      | Jordan, Jr. et al. |                |  |
| 4,714,116 A           | 12/1987          | Brunner               | 5,435,392 A   | 7/1995      | Kennedy            |                |  |
| 4,721,159 A           | 1/1988           | Ohkochi et al.        | 5,439,051 A   | 8/1995      | Kennedy et al.     |                |  |
| 4,738,599 A           | 4/1988           | Shilling              | 5,454,430 A   | 10/1995     | Kennedy et al.     |                |  |
| 4,768,588 A           | 9/1988           | Kupsa                 | 5,456,317 A   | 10/1995     | Hood, III et al.   |                |  |
| 4,775,598 A           | 10/1988          | Jaekel                | 5,464,062 A   | 11/1995     | Blizzard, Jr.      |                |  |
| 4,784,226 A           | 11/1988          | Wyatt                 | 5,472,048 A   | 12/1995     | Kennedy et al.     |                |  |
| 4,805,699 A           | 2/1989           | Halbardier            | 5,474,131 A   | 12/1995     | Jordan, Jr. et al. |                |  |
| 4,817,725 A           | 4/1989           | Jenkins               | 5,477,923 A   | 12/1995     | Jordan, Jr. et al. |                |  |
| 4,834,184 A           | 5/1989           | Streich et al.        | 5,507,439 A   | 4/1996      | Story              |                |  |
| H635 H                | 6/1989           | Johnson et al.        | 5,526,880 A   | 6/1996      | Jordan, Jr. et al. |                |  |
| 4,850,432 A           | 7/1989           | Porter et al.         | 5,526,881 A   | 6/1996      | Martin et al.      |                |  |
| 4,853,056 A           | 8/1989           | Hoffman               | 5,529,746 A   | 6/1996      | Knoss et al.       |                |  |
| 4,869,324 A           | 9/1989           | Holder                | 5,533,573 A   | 7/1996      | Jordan, Jr. et al. |                |  |
| 4,869,325 A           | 9/1989           | Halbardier            | 5,536,485 A   | 7/1996      | Kume et al.        |                |  |
| 4,889,187 A           | 12/1989          | Terrell et al.        | 5,558,153 A   | 9/1996      | Holcombe et al.    |                |  |
| 4,890,675 A           | 1/1990           | Dew                   | 5,607,017 A * | 3/1997      | Owens et al. ..... | 166/288        |  |
| 4,909,320 A           | 3/1990           | Hebert et al.         | 5,623,993 A   | 4/1997      | Van Buskirk et al. |                |  |
| 4,929,415 A           | 5/1990           | Okazaki               | 5,623,994 A   | 4/1997      | Robinson           |                |  |
| 4,932,474 A           | 6/1990           | Schroeder, Jr. et al. | 5,636,691 A   | 6/1997      | Hendrickson et al. |                |  |
| 4,938,309 A           | 7/1990           | Emdy                  | 5,641,023 A   | 6/1997      | Ross et al.        |                |  |
| 4,938,809 A           | 7/1990           | Das et al.            | 5,647,444 A   | 7/1997      | Williams           |                |  |
| 4,944,351 A           | 7/1990           | Eriksen et al.        | 5,665,289 A   | 9/1997      | Chung et al.       |                |  |
| 4,949,788 A           | 8/1990           | Szarka et al.         | 5,677,372 A   | 10/1997     | Yamamoto et al.    |                |  |
| 4,952,902 A           | 8/1990           | Kawaguchi et al.      | 5,685,372 A   | 11/1997     | Gano               |                |  |
| 4,975,412 A           | 12/1990          | Okazaki et al.        | 5,701,576 A   | 12/1997     | Fujita et al.      |                |  |
| 4,977,958 A           | 12/1990          | Miller                | 5,707,214 A   | 1/1998      | Schmidt            |                |  |
| 4,981,177 A           | 1/1991           | Carmody et al.        | 5,709,269 A   | 1/1998      | Head               |                |  |
| 4,986,361 A           | 1/1991           | Mueller et al.        | 5,720,344 A   | 2/1998      | Newman             |                |  |
| 4,997,622 A           | 3/1991           | Regazzoni et al.      | 5,728,195 A   | 3/1998      | Eastman et al.     |                |  |
| 5,006,044 A           | 4/1991           | Walker, Sr. et al.    | 5,765,639 A   | 6/1998      | Muth               |                |  |
| 5,010,955 A           | 4/1991           | Springer              | 5,772,735 A   | 6/1998      | Sehgal et al.      |                |  |
| 5,036,921 A           | 8/1991           | Pittard et al.        | 5,782,305 A   | 7/1998      | Hicks              |                |  |
| 5,048,611 A           | 9/1991           | Cochran               | 5,797,454 A   | 8/1998      | Hipp               |                |  |
| 5,049,165 A           | 9/1991           | Tselesin              | 5,826,652 A   | 10/1998     | Tapp               |                |  |
|                       |                  |                       | 5,826,661 A   | 10/1998     | Parker et al.      |                |  |
|                       |                  |                       | 5,829,520 A   | 11/1998     | Johnson            |                |  |
|                       |                  |                       | 5,836,396 A   | 11/1998     | Norman             |                |  |
|                       |                  |                       | 5,857,521 A   | 1/1999      | Ross et al.        |                |  |

(56)

## References Cited

## U.S. PATENT DOCUMENTS

|              |         |                    |              |         |                      |
|--------------|---------|--------------------|--------------|---------|----------------------|
| 5,881,816 A  | 3/1999  | Wright             | 6,613,383 B1 | 9/2003  | George et al.        |
| 5,896,819 A  | 4/1999  | Turila et al.      | 6,619,400 B2 | 9/2003  | Brunet               |
| 5,902,424 A  | 5/1999  | Fujita et al.      | 6,634,428 B2 | 10/2003 | Krauss et al.        |
| 5,934,372 A  | 8/1999  | Muth               | 6,662,886 B2 | 12/2003 | Russell              |
| 5,960,881 A  | 10/1999 | Allamont et al.    | 6,675,889 B1 | 1/2004  | Mullins et al.       |
| 5,990,051 A  | 11/1999 | Ischy et al.       | 6,699,305 B2 | 3/2004  | Myrick               |
| 5,992,452 A  | 11/1999 | Nelson, II         | 6,713,177 B2 | 3/2004  | George et al.        |
| 5,992,520 A  | 11/1999 | Schultz et al.     | 6,715,541 B2 | 4/2004  | Pedersen et al.      |
| 6,007,314 A  | 12/1999 | Nelson, II         | 6,719,051 B2 | 4/2004  | Hailey, Jr. et al.   |
| 6,024,915 A  | 2/2000  | Kume et al.        | 6,755,249 B2 | 6/2004  | Robison et al.       |
| 6,032,735 A  | 3/2000  | Echols             | 6,776,228 B2 | 8/2004  | Pedersen et al.      |
| 6,036,777 A  | 3/2000  | Sachs              | 6,779,599 B2 | 8/2004  | Mullins et al.       |
| 6,047,773 A  | 4/2000  | Zeltmann et al.    | 6,799,638 B2 | 10/2004 | Butterfield, Jr.     |
| 6,050,340 A  | 4/2000  | Scott              | 6,810,960 B2 | 11/2004 | Pia                  |
| 6,069,313 A  | 5/2000  | Kay                | 6,817,414 B2 | 11/2004 | Lee                  |
| 6,076,600 A  | 6/2000  | Vick, Jr. et al.   | 6,831,044 B2 | 12/2004 | Constien             |
| 6,079,496 A  | 6/2000  | Hirth              | 6,883,611 B2 | 4/2005  | Smith et al.         |
| 6,085,837 A  | 7/2000  | Massinon et al.    | 6,887,297 B2 | 5/2005  | Winter et al.        |
| 6,095,247 A  | 8/2000  | Streich et al.     | 6,896,049 B2 | 5/2005  | Moyes                |
| 6,119,783 A  | 9/2000  | Parker et al.      | 6,896,061 B2 | 5/2005  | Hriscu et al.        |
| 6,142,237 A  | 11/2000 | Christmas et al.   | 6,899,176 B2 | 5/2005  | Hailey, Jr. et al.   |
| 6,161,622 A  | 12/2000 | Robb et al.        | 6,932,159 B2 | 8/2005  | Hovem                |
| 6,167,970 B1 | 1/2001  | Stout et al.       | 6,945,331 B2 | 9/2005  | Patel                |
| 6,170,583 B1 | 1/2001  | Boyce              | 6,951,331 B2 | 10/2005 | Haughom et al.       |
| 6,173,779 B1 | 1/2001  | Smith              | 6,959,759 B2 | 11/2005 | Doane et al.         |
| 6,189,616 B1 | 2/2001  | Gano et al.        | 6,973,970 B2 | 12/2005 | Johnston et al.      |
| 6,213,202 B1 | 4/2001  | Read, Jr.          | 6,973,973 B2 | 12/2005 | Howard et al.        |
| 6,220,350 B1 | 4/2001  | Brothers et al.    | 6,983,796 B2 | 1/2006  | Bayne et al.         |
| 6,220,357 B1 | 4/2001  | Carmichael         | 6,986,390 B2 | 1/2006  | Doane et al.         |
| 6,228,904 B1 | 5/2001  | Yadav et al.       | 7,013,989 B2 | 3/2006  | Hammond et al.       |
| 6,237,688 B1 | 5/2001  | Burleson et al.    | 7,017,664 B2 | 3/2006  | Walker et al.        |
| 6,238,280 B1 | 5/2001  | Ritt et al.        | 7,017,677 B2 | 3/2006  | Keshavan et al.      |
| 6,241,021 B1 | 6/2001  | Bowling            | 7,021,389 B2 | 4/2006  | Bishop et al.        |
| 6,248,399 B1 | 6/2001  | Hehmann            | 7,025,146 B2 | 4/2006  | King et al.          |
| 6,250,392 B1 | 6/2001  | Muth               | 7,028,778 B2 | 4/2006  | Krywitsky            |
| 6,273,187 B1 | 8/2001  | Voisin, Jr. et al. | 7,044,230 B2 | 5/2006  | Starr et al.         |
| 6,276,452 B1 | 8/2001  | Davis et al.       | 7,049,272 B2 | 5/2006  | Sinclair et al.      |
| 6,276,457 B1 | 8/2001  | Moffatt et al.     | 7,051,805 B2 | 5/2006  | Doane et al.         |
| 6,279,656 B1 | 8/2001  | Sinclair et al.    | 7,059,410 B2 | 6/2006  | Bousche et al.       |
| 6,287,445 B1 | 9/2001  | Lashmore et al.    | 7,090,027 B1 | 8/2006  | Williams             |
| 6,302,205 B1 | 10/2001 | Ryll               | 7,093,664 B2 | 8/2006  | Todd et al.          |
| 6,315,041 B1 | 11/2001 | Carlisle et al.    | 7,096,945 B2 | 8/2006  | Richards et al.      |
| 6,315,050 B2 | 11/2001 | Vaynshteyn et al.  | 7,096,946 B2 | 8/2006  | Jasser et al.        |
| 6,325,148 B1 | 12/2001 | Trahan et al.      | 7,097,906 B2 | 8/2006  | Gardner              |
| 6,328,110 B1 | 12/2001 | Joubert            | 7,108,080 B2 | 9/2006  | Tessari et al.       |
| 6,341,653 B1 | 1/2002  | Firmaniuk et al.   | 7,111,682 B2 | 9/2006  | Blaisdell            |
| 6,349,766 B1 | 2/2002  | Bussear et al.     | 7,141,207 B2 | 11/2006 | Jandeska, Jr. et al. |
| 6,354,379 B2 | 3/2002  | Miszewski et al.   | 7,150,326 B2 | 12/2006 | Bishop et al.        |
| 6,357,322 B1 | 3/2002  | Dolan              | 7,163,066 B2 | 1/2007  | Lehr                 |
| 6,357,332 B1 | 3/2002  | Vecchio            | 7,174,963 B2 | 2/2007  | Bertelsen            |
| 6,371,206 B1 | 4/2002  | Mills              | 7,182,135 B2 | 2/2007  | Szarka               |
| 6,372,346 B1 | 4/2002  | Toth               | 7,188,559 B1 | 3/2007  | Vecchio              |
| 6,382,244 B2 | 5/2002  | Vann               | 7,210,527 B2 | 5/2007  | Walker et al.        |
| 6,390,195 B1 | 5/2002  | Nguyen et al.      | 7,210,533 B2 | 5/2007  | Starr et al.         |
| 6,390,200 B1 | 5/2002  | Allamont et al.    | 7,217,311 B2 | 5/2007  | Hong et al.          |
| 6,394,185 B1 | 5/2002  | Constien           | 7,234,530 B2 | 6/2007  | Gass                 |
| 6,397,950 B1 | 6/2002  | Streich et al.     | 7,252,162 B2 | 8/2007  | Akinlade et al.      |
| 6,408,946 B1 | 6/2002  | Marshall et al.    | 7,255,172 B2 | 8/2007  | Johnson              |
| 6,419,023 B1 | 7/2002  | George et al.      | 7,255,178 B2 | 8/2007  | Slup et al.          |
| 6,439,313 B1 | 8/2002  | Thomeer et al.     | 7,264,060 B2 | 9/2007  | Wills                |
| 6,457,525 B1 | 10/2002 | Scott              | 7,267,172 B2 | 9/2007  | Hofman               |
| 6,467,546 B2 | 10/2002 | Allamont et al.    | 7,267,178 B2 | 9/2007  | Krywitsky            |
| 6,470,965 B1 | 10/2002 | Winzer             | 7,270,186 B2 | 9/2007  | Johnson              |
| 6,491,097 B1 | 12/2002 | O'Neal et al.      | 7,287,592 B2 | 10/2007 | Surjaatmadja et al.  |
| 6,491,116 B2 | 12/2002 | Berscheidt et al.  | 7,311,152 B2 | 12/2007 | Howard et al.        |
| 6,513,598 B2 | 2/2003  | Moore et al.       | 7,316,274 B2 | 1/2008  | Xu et al.            |
| 6,540,033 B1 | 4/2003  | Sullivan et al.    | 7,320,365 B2 | 1/2008  | Pia                  |
| 6,543,543 B2 | 4/2003  | Muth               | 7,322,412 B2 | 1/2008  | Badalamenti et al.   |
| 6,561,275 B2 | 5/2003  | Glass et al.       | 7,322,417 B2 | 1/2008  | Rytlewski et al.     |
| 6,588,507 B2 | 7/2003  | Dusterhoff et al.  | 7,325,617 B2 | 2/2008  | Murray               |
| 6,591,915 B2 | 7/2003  | Burris et al.      | 7,328,750 B2 | 2/2008  | Swor et al.          |
| 6,601,648 B2 | 8/2003  | Ebinger            | 7,331,388 B2 | 2/2008  | Vilela et al.        |
| 6,601,650 B2 | 8/2003  | Sundararajan       | 7,337,854 B2 | 3/2008  | Horn et al.          |
| 6,609,569 B2 | 8/2003  | Howlett et al.     | 7,346,456 B2 | 3/2008  | Le Bemadjiel         |
| 6,612,826 B1 | 9/2003  | Bauer et al.       | 7,360,593 B2 | 4/2008  | Constien             |

| (56)                  | References Cited                |                 |                             |  |  |
|-----------------------|---------------------------------|-----------------|-----------------------------|--|--|
| U.S. PATENT DOCUMENTS |                                 |                 |                             |  |  |
| 7,360,597 B2          | 4/2008 Blaisdell                | 7,909,096 B2    | 3/2011 Clark et al.         |  |  |
| 7,384,443 B2          | 6/2008 Mirchandani              | 7,909,104 B2    | 3/2011 Bjorgum              |  |  |
| 7,387,158 B2          | 6/2008 Murray et al.            | 7,909,110 B2    | 3/2011 Sharma et al.        |  |  |
| 7,387,165 B2          | 6/2008 Lopez de Cardenas et al. | 7,909,115 B2    | 3/2011 Grove et al.         |  |  |
| 7,392,841 B2          | 7/2008 Murray et al.            | 7,913,765 B2    | 3/2011 Crow et al.          |  |  |
| 7,401,648 B2          | 7/2008 Richard                  | 7,931,093 B2    | 4/2011 Foster et al.        |  |  |
| 7,416,029 B2          | 8/2008 Telfer et al.            | 7,938,191 B2    | 5/2011 Vaidya               |  |  |
| 7,422,058 B2          | 9/2008 O'Malley                 | 7,946,335 B2    | 5/2011 Bewlay et al.        |  |  |
| 7,426,964 B2          | 9/2008 Lynde et al.             | 7,946,340 B2    | 5/2011 Surjaatmadja et al.  |  |  |
| 7,441,596 B2          | 10/2008 Wood et al.             | 7,980,300 B2    | 7/2011 Roberts et al.       |  |  |
| 7,445,049 B2          | 11/2008 Howard et al.           | 7,987,906 B1    | 8/2011 Troy                 |  |  |
| 7,451,815 B2          | 11/2008 Hailey, Jr.             | 7,992,763 B2    | 8/2011 Vecchio et al.       |  |  |
| 7,451,817 B2          | 11/2008 Reddy et al.            | 8,020,619 B1    | 9/2011 Robertson et al.     |  |  |
| 7,461,699 B2          | 12/2008 Richard et al.          | 8,020,620 B2    | 9/2011 Daniels et al.       |  |  |
| 7,464,764 B2          | 12/2008 Xu                      | 8,025,104 B2    | 9/2011 Cooke, Jr.           |  |  |
| 7,472,750 B2          | 1/2009 Walker et al.            | 8,028,767 B2    | 10/2011 Radford et al.      |  |  |
| 7,478,676 B2          | 1/2009 East, Jr. et al.         | 8,033,331 B2    | 10/2011 Themig              |  |  |
| 7,503,390 B2          | 3/2009 Gomez                    | 8,039,422 B1    | 10/2011 Al-Zahrani          |  |  |
| 7,503,399 B2          | 3/2009 Badalamenti et al.       | 8,056,628 B2    | 11/2011 Whitsitt et al.     |  |  |
| 7,510,018 B2          | 3/2009 Williamson et al.        | 8,056,638 B2    | 11/2011 Clayton et al.      |  |  |
| 7,513,311 B2          | 4/2009 Gramstad et al.          | 8,109,340 B2    | 2/2012 Doane et al.         |  |  |
| 7,527,103 B2          | 5/2009 Huang et al.             | 8,127,856 B1    | 3/2012 Nish et al.          |  |  |
| 7,537,825 B1          | 5/2009 Wardle et al.            | 8,153,052 B2    | 4/2012 Jackson et al.       |  |  |
| 7,552,777 B2          | 6/2009 Murray et al.            | 8,163,060 B2    | 4/2012 Imanishi et al.      |  |  |
| 7,552,779 B2          | 6/2009 Murray                   | 8,211,247 B2    | 7/2012 Marya et al.         |  |  |
| 7,575,062 B2          | 8/2009 East, Jr.                | 8,211,248 B2    | 7/2012 Marya                |  |  |
| 7,591,318 B2          | 9/2009 Tilghman                 | 8,226,740 B2    | 7/2012 Chaumonnot et al.    |  |  |
| 7,600,572 B2          | 10/2009 Slup et al.             | 8,230,731 B2    | 7/2012 Dyer et al.          |  |  |
| 7,604,055 B2          | 10/2009 Richard et al.          | 8,231,947 B2    | 7/2012 Vaidya et al.        |  |  |
| 7,617,871 B2          | 11/2009 Surjaatmadja et al.     | 8,276,670 B2    | 10/2012 Patel               |  |  |
| 7,635,023 B2          | 12/2009 Goldberg et al.         | 8,277,974 B2    | 10/2012 Kumar et al.        |  |  |
| 7,640,988 B2          | 1/2010 Phi et al.               | 8,297,364 B2    | 10/2012 Agrawal et al.      |  |  |
| 7,661,480 B2          | 2/2010 Al-Anazi                 | 8,327,931 B2    | 12/2012 Agrawal et al.      |  |  |
| 7,661,481 B2          | 2/2010 Todd et al.              | 8,403,037 B2    | 3/2013 Agrawal et al.       |  |  |
| 7,665,537 B2          | 2/2010 Patel et al.             | 8,425,651 B2    | 4/2013 Xu et al.            |  |  |
| 7,686,082 B2          | 3/2010 Marsh                    | 2001/0045285 A1 | 11/2001 Russell             |  |  |
| 7,690,436 B2          | 4/2010 Turley et al.            | 2001/0045288 A1 | 11/2001 Allamon et al.      |  |  |
| 7,699,101 B2          | 4/2010 Fripp et al.             | 2002/0000319 A1 | 1/2002 Brunet               |  |  |
| 7,703,510 B2          | 4/2010 Xu                       | 2002/007948 A1  | 1/2002 Bayne et al.         |  |  |
| 7,703,511 B2          | 4/2010 Buyers et al.            | 2002/0014268 A1 | 2/2002 Vann                 |  |  |
| 7,708,078 B2          | 5/2010 Stoesz                   | 2002/0066572 A1 | 6/2002 Muth                 |  |  |
| 7,709,421 B2          | 5/2010 Jones et al.             | 2002/0104616 A1 | 8/2002 De et al.            |  |  |
| 7,712,541 B2          | 5/2010 Loretz et al.            | 2002/0136904 A1 | 9/2002 Glass et al.         |  |  |
| 7,723,272 B2          | 5/2010 Crews et al.             | 2002/0162661 A1 | 11/2002 Krauss et al.       |  |  |
| 7,726,406 B2          | 6/2010 Xu                       | 2003/0037925 A1 | 2/2003 Walker et al.        |  |  |
| 7,735,578 B2          | 6/2010 Loehr et al.             | 2003/0060374 A1 | 3/2003 Cooke, Jr.           |  |  |
| 7,752,971 B2          | 7/2010 Loehr                    | 2003/0075326 A1 | 4/2003 Ebinger              |  |  |
| 7,757,773 B2          | 7/2010 Rytlewski                | 2003/0104147 A1 | 6/2003 Bretschneider et al. |  |  |
| 7,762,342 B2          | 7/2010 Richard et al.           | 2003/0111728 A1 | 6/2003 Thai et al.          |  |  |
| 7,770,652 B2          | 8/2010 Barnett                  | 2003/0127013 A1 | 7/2003 Zavitsanos et al.    |  |  |
| 7,775,284 B2          | 8/2010 Richards et al.          | 2003/0141060 A1 | 7/2003 Hailey et al.        |  |  |
| 7,775,285 B2          | 8/2010 Surjaatmadja et al.      | 2003/0141061 A1 | 7/2003 Hailey et al.        |  |  |
| 7,775,286 B2 *        | 8/2010 Duphorne ..... 166/376   | 2003/0141079 A1 | 7/2003 Doane et al.         |  |  |
| 7,784,543 B2          | 8/2010 Johnson                  | 2003/0150614 A1 | 8/2003 Brown et al.         |  |  |
| 7,793,714 B2          | 9/2010 Johnson                  | 2003/0155114 A1 | 8/2003 Pedersen et al.      |  |  |
| 7,798,225 B2          | 9/2010 Giroux et al.            | 2003/0155115 A1 | 8/2003 Pedersen et al.      |  |  |
| 7,798,226 B2          | 9/2010 Themig                   | 2003/0159828 A1 | 8/2003 Howard et al.        |  |  |
| 7,798,236 B2          | 9/2010 McKeachnie et al.        | 2003/0164237 A1 | 9/2003 Butterfield          |  |  |
| 7,806,189 B2          | 10/2010 Frazier                 | 2003/0183391 A1 | 10/2003 Hriscu et al.       |  |  |
| 7,806,192 B2          | 10/2010 Foster et al.           | 2004/0005483 A1 | 1/2004 Lin                  |  |  |
| 7,810,553 B2          | 10/2010 Cruickshank et al.      | 2004/0020832 A1 | 2/2004 Richards et al.      |  |  |
| 7,810,567 B2          | 10/2010 Daniels et al.          | 2004/0031605 A1 | 2/2004 Mickey               |  |  |
| 7,819,198 B2          | 10/2010 Birckhead et al.        | 2004/0045723 A1 | 3/2004 Slup et al.          |  |  |
| 7,828,055 B2          | 11/2010 Willauer et al.         | 2004/0055758 A1 | 3/2004 Brezinski et al.     |  |  |
| 7,833,944 B2          | 11/2010 Munoz et al.            | 2004/0089449 A1 | 5/2004 Walton et al.        |  |  |
| 7,849,927 B2          | 12/2010 Herrera                 | 2004/0154806 A1 | 8/2004 Bode et al.          |  |  |
| 7,855,168 B2          | 12/2010 Fuller et al.           | 2004/0159428 A1 | 8/2004 Hammond et al.       |  |  |
| 7,861,779 B2          | 1/2011 Vestavik                 | 2004/0182583 A1 | 9/2004 Doane et al.         |  |  |
| 7,861,781 B2          | 1/2011 D'Arcy                   | 2004/0256109 A1 | 12/2004 Johnson             |  |  |
| 7,874,365 B2          | 1/2011 East, Jr. et al.         | 2004/0256157 A1 | 12/2004 Tessari et al.      |  |  |
| 7,878,253 B2          | 2/2011 Stowe et al.             | 2004/0261993 A1 | 12/2004 Nguyen              |  |  |
| 7,896,091 B2          | 3/2011 Williamson et al.        | 2005/0034876 A1 | 2/2005 Doane et al.         |  |  |
| 7,897,063 B1          | 3/2011 Perry et al.             | 2005/0051329 A1 | 3/2005 Blaisdell            |  |  |
| 7,900,696 B1          | 3/2011 Nish et al.              | 2005/0064247 A1 | 3/2005 Sane et al.          |  |  |
| 7,900,703 B2          | 3/2011 Clark et al.             | 2005/0069449 A1 | 3/2005 Jackson et al.       |  |  |

| (56)                  | References Cited  |                                  |
|-----------------------|-------------------|----------------------------------|
| U.S. PATENT DOCUMENTS |                   |                                  |
| 2005/0102255 A1       | 5/2005            | Bultman                          |
| 2005/0106316 A1       | 5/2005            | Rigney et al.                    |
| 2005/0126334 A1       | 6/2005            | Mirchandani                      |
| 2005/0161224 A1       | 7/2005            | Starr et al.                     |
| 2005/0165149 A1       | 7/2005            | Chanak et al.                    |
| 2005/0194143 A1       | 9/2005            | Xu et al.                        |
| 2005/0199401 A1       | 9/2005            | Patel et al.                     |
| 2005/0205264 A1 *     | 9/2005            | Starr et al. .... 166/376        |
| 2005/0205266 A1       | 9/2005            | Todd et al.                      |
| 2005/0241824 A1       | 11/2005           | Burris, II et al.                |
| 2005/0241825 A1       | 11/2005           | Burris, II et al.                |
| 2005/0257936 A1       | 11/2005           | Lehr                             |
| 2005/0279501 A1       | 12/2005           | Surjaatmadja et al.              |
| 2006/0012087 A1       | 1/2006            | Matsuda et al.                   |
| 2006/0045787 A1       | 3/2006            | Jandeska, Jr. et al.             |
| 2006/0057479 A1       | 3/2006            | Niimi et al.                     |
| 2006/0081378 A1       | 4/2006            | Howard et al.                    |
| 2006/0102871 A1       | 5/2006            | Wang et al.                      |
| 2006/0108114 A1       | 5/2006            | Johnson et al.                   |
| 2006/0108126 A1       | 5/2006            | Horn et al.                      |
| 2006/0116696 A1       | 6/2006            | Odermatt et al.                  |
| 2006/0124310 A1       | 6/2006            | Lopez de Cardenas                |
| 2006/0124312 A1       | 6/2006            | Rytlewski et al.                 |
| 2006/0131011 A1       | 6/2006            | Lynde et al.                     |
| 2006/0131081 A1       | 6/2006            | Mirchandani et al.               |
| 2006/0144515 A1       | 7/2006            | Tada et al.                      |
| 2006/0150770 A1       | 7/2006            | Freim, III et al.                |
| 2006/0151178 A1       | 7/2006            | Howard et al.                    |
| 2006/0162927 A1       | 7/2006            | Walker et al.                    |
| 2006/0169453 A1       | 8/2006            | Savery et al.                    |
| 2006/0207763 A1       | 9/2006            | Hofman et al.                    |
| 2006/0213670 A1       | 9/2006            | Bishop et al.                    |
| 2006/0231253 A1       | 10/2006           | Vilela et al.                    |
| 2006/0283592 A1       | 12/2006           | Sierra et al.                    |
| 2007/00117674 A1      | 1/2007            | Blaisdell                        |
| 2007/00117675 A1      | 1/2007            | Hammami et al.                   |
| 2007/0029082 A1       | 2/2007            | Giroux et al.                    |
| 2007/0039741 A1       | 2/2007            | Hailey                           |
| 2007/0029082 A1       | 2/2007            | Giroux et al.                    |
| 2007/0044966 A1       | 3/2007            | Davies et al.                    |
| 2007/0051521 A1       | 3/2007            | Fike et al.                      |
| 2007/0053785 A1       | 3/2007            | Hetz et al.                      |
| 2007/0054101 A1       | 3/2007            | Sigalas et al.                   |
| 2007/0057415 A1       | 3/2007            | Katagiri et al.                  |
| 2007/0062644 A1       | 3/2007            | Nakamura et al.                  |
| 2007/0074601 A1       | 4/2007            | Hong et al.                      |
| 2007/0074873 A1       | 4/2007            | McKeachnie et al.                |
| 2007/0102199 A1       | 5/2007            | Smith et al.                     |
| 2007/0107899 A1       | 5/2007            | Werner et al.                    |
| 2007/0107908 A1 *     | 5/2007            | Vaidya et al. .... 166/376       |
| 2007/0108060 A1       | 5/2007            | Park                             |
| 2007/0119600 A1       | 5/2007            | Slup et al.                      |
| 2007/0131912 A1       | 6/2007            | Simone et al.                    |
| 2007/0151009 A1       | 7/2007            | Conrad, III et al.               |
| 2007/0151769 A1       | 7/2007            | Slutz et al.                     |
| 2007/0169935 A1       | 7/2007            | Akbar et al.                     |
| 2007/0181224 A1 *     | 8/2007            | Marya et al. .... 148/400        |
| 2007/0185655 A1       | 8/2007            | Le Bemadjiel                     |
| 2007/0187095 A1       | 8/2007            | Walker et al.                    |
| 2007/0221373 A1       | 9/2007            | Murray                           |
| 2007/0221384 A1       | 9/2007            | Murray                           |
| 2007/0261862 A1       | 11/2007           | Murray                           |
| 2007/0272411 A1       | 11/2007           | Lopez De Cardenas et al.         |
| 2007/0272413 A1       | 11/2007           | Rytlewski et al.                 |
| 2007/0277979 A1       | 12/2007           | Todd et al.                      |
| 2007/0284109 A1       | 12/2007           | East et al.                      |
| 2007/0284112 A1       | 12/2007           | Magne et al.                     |
| 2007/0299510 A1       | 12/2007           | Venkatarman et al.               |
| 2008/0011473 A1       | 1/2008            | Wood et al.                      |
| 2008/0020923 A1       | 1/2008            | Debe et al.                      |
| 2008/0047707 A1       | 2/2008            | Boney et al.                     |
| 2008/0060810 A9       | 3/2008            | Nguyen et al.                    |
| 2008/0066923 A1 *     | 3/2008            | Xu .... 166/376                  |
| 2008/0066924 A1       | 3/2008            | Xu                               |
| 2008/0072705 A1       | 3/2008            | Chaumonnot et al.                |
|                       | 2008/0078553 A1   | 4/2008 George                    |
|                       | 2008/0099209 A1   | 5/2008 Loretz et al.             |
|                       | 2008/0115932 A1   | 5/2008 Cooke                     |
|                       | 2008/0121390 A1   | 5/2008 O'Malley et al.           |
|                       | 2008/0135249 A1   | 6/2008 Fripp et al.              |
|                       | 2008/0149325 A1   | 6/2008 Crawford                  |
|                       | 2008/0149345 A1 * | 6/2008 Marya et al. .... 166/376 |
|                       | 2008/0169105 A1   | 7/2008 Williamson et al.         |
|                       | 2008/0179060 A1   | 7/2008 Surjaatmadja et al.       |
|                       | 2008/0179104 A1   | 7/2008 Zhang et al.              |
|                       | 2008/0202764 A1   | 8/2008 Clayton et al.            |
|                       | 2008/0202814 A1   | 8/2008 Lyons et al.              |
|                       | 2008/0210473 A1   | 9/2008 Zhang et al.              |
|                       | 2008/0216383 A1   | 9/2008 Pierick et al.            |
|                       | 2008/0223586 A1   | 9/2008 Barnett                   |
|                       | 2008/0223587 A1   | 9/2008 Cherewyk                  |
|                       | 2008/0236829 A1   | 10/2008 Lynde                    |
|                       | 2008/0248205 A1   | 10/2008 Blanchet et al.          |
|                       | 2008/0277109 A1   | 11/2008 Vaidya                   |
|                       | 2008/0277980 A1   | 11/2008 Koda et al.              |
|                       | 2008/0282924 A1   | 11/2008 Saenger et al.           |
|                       | 2008/0296024 A1   | 12/2008 Huang et al.             |
|                       | 2008/0314581 A1   | 12/2008 Brown                    |
|                       | 2008/0314588 A1   | 12/2008 Langlais et al.          |
|                       | 2009/0044946 A1   | 2/2009 Schasteen et al.          |
|                       | 2009/0044949 A1   | 2/2009 King et al.               |
|                       | 2009/0050334 A1   | 2/2009 Marya et al.              |
|                       | 2009/0056934 A1   | 3/2009 Xu                        |
|                       | 2009/0065216 A1   | 3/2009 Frazier                   |
|                       | 2009/0084550 A1   | 4/2009 Korte et al.              |
|                       | 2009/0084553 A1   | 4/2009 Rytlewski et al.          |
|                       | 2009/0084556 A1   | 4/2009 Richards et al.           |
|                       | 2009/0090440 A1   | 4/2009 Kellett et al.            |
|                       | 2009/0107684 A1   | 4/2009 Cooke, Jr.                |
|                       | 2009/0114381 A1   | 5/2009 Stroobants                |
|                       | 2009/0114382 A1   | 5/2009 Grove et al.              |
|                       | 2009/0145666 A1   | 6/2009 Radford et al.            |
|                       | 2009/0151949 A1   | 6/2009 Marya et al.              |
|                       | 2009/0155616 A1   | 6/2009 Thamida et al.            |
|                       | 2009/0159289 A1   | 6/2009 Avant et al.              |
|                       | 2009/0178808 A1   | 7/2009 Williamson et al.         |
|                       | 2009/0194273 A1   | 8/2009 Surjaatmadja et al.       |
|                       | 2009/0205841 A1   | 8/2009 Kluge et al.              |
|                       | 2009/0226704 A1   | 9/2009 Kauppinen et al.          |
|                       | 2009/0242202 A1   | 10/2009 Rispler et al.           |
|                       | 2009/0242208 A1   | 10/2009 Bolding                  |
|                       | 2009/0242214 A1   | 10/2009 Foster et al.            |
|                       | 2009/0255667 A1   | 10/2009 Clem et al.              |
|                       | 2009/0255684 A1   | 10/2009 Bolding                  |
|                       | 2009/0255686 A1   | 10/2009 Richard et al.           |
|                       | 2009/0260817 A1   | 10/2009 Gambier et al.           |
|                       | 2009/0266548 A1   | 10/2009 Olsen et al.             |
|                       | 2009/0272544 A1   | 11/2009 Giroux et al.            |
|                       | 2009/0283270 A1   | 11/2009 Langeslag                |
|                       | 2009/0293672 A1   | 12/2009 Mirchandani et al.       |
|                       | 2009/0301730 A1   | 12/2009 Gweily                   |
|                       | 2009/0305131 A1   | 12/2009 Kumar et al.             |
|                       | 2009/0308588 A1   | 12/2009 Howell et al.            |
|                       | 2009/0317556 A1   | 12/2009 Macary                   |
|                       | 2010/0003536 A1   | 1/2010 Smith et al.              |
|                       | 2010/0012385 A1   | 1/2010 Drivdahl et al.           |
|                       | 2010/0015469 A1   | 1/2010 Romanowski et al.         |
|                       | 2010/0025255 A1 * | 2/2010 Su et al. .... 205/176    |
|                       | 2010/0032151 A1 * | 2/2010 Duphorne .... 166/55      |
|                       | 2010/0040180 A1   | 2/2010 Kim et al.                |
|                       | 2010/0044041 A1   | 2/2010 Smith et al.              |
|                       | 2010/0051278 A1   | 3/2010 Mytopher et al.           |
|                       | 2010/0055491 A1   | 3/2010 Vecchio et al.            |
|                       | 2010/0055492 A1   | 3/2010 Barsoum et al.            |
|                       | 2010/0089583 A1   | 4/2010 Xu et al.                 |
|                       | 2010/0089587 A1   | 4/2010 Stout                     |
|                       | 2010/0101803 A1   | 4/2010 Clayton et al.            |
|                       | 2010/0122817 A1   | 5/2010 Surjaatmadja et al.       |
|                       | 2010/0139930 A1   | 6/2010 Patel et al.              |
|                       | 2010/0200230 A1   | 8/2010 East, Jr. et al.          |
|                       | 2010/0236793 A1   | 9/2010 Bjorgum                   |
|                       | 2010/0236794 A1   | 9/2010 Duan et al.               |
|                       | 2010/0243254 A1   | 9/2010 Murphy et al.             |
|                       | 2010/0252273 A1   | 10/2010 Duphorne                 |

| (56)                     | References Cited |                          |                                                                                                                                                                                                                                                                                                                                                                                                  |               |         |  |
|--------------------------|------------------|--------------------------|--------------------------------------------------------------------------------------------------------------------------------------------------------------------------------------------------------------------------------------------------------------------------------------------------------------------------------------------------------------------------------------------------|---------------|---------|--|
| U.S. PATENT DOCUMENTS    |                  |                          |                                                                                                                                                                                                                                                                                                                                                                                                  |               |         |  |
| 2010/0252280 A1          | 10/2010          | Swor et al.              | WO                                                                                                                                                                                                                                                                                                                                                                                               | 9947726 A1    | 9/1999  |  |
| 2010/0270031 A1          | 10/2010          | Patel                    | WO                                                                                                                                                                                                                                                                                                                                                                                               | 2008034042 A2 | 3/2008  |  |
| 2010/0276136 A1          | 11/2010          | Evans et al.             | WO                                                                                                                                                                                                                                                                                                                                                                                               | 2008079777 A3 | 7/2008  |  |
| 2010/0282338 A1          | 11/2010          | Gerrard et al.           | WO                                                                                                                                                                                                                                                                                                                                                                                               | WO2008079485  | 7/2008  |  |
| 2010/0282469 A1          | 11/2010          | Richard et al.           | WO                                                                                                                                                                                                                                                                                                                                                                                               | 2009079745 A1 | 7/2009  |  |
| 2010/0294510 A1          | 11/2010          | Holmes                   | WO                                                                                                                                                                                                                                                                                                                                                                                               | 2011071902 A3 | 6/2011  |  |
| 2010/0319870 A1          | 12/2010          | Bewlay et al.            | WO                                                                                                                                                                                                                                                                                                                                                                                               | 2011071910 A2 | 6/2011  |  |
| 2011/0005773 A1          | 1/2011           | Dusterhoft et al.        | WO                                                                                                                                                                                                                                                                                                                                                                                               | 2011071910 A3 | 6/2011  |  |
| 2011/0036592 A1          | 2/2011           | Fay                      | WO                                                                                                                                                                                                                                                                                                                                                                                               | 2012174101 A2 | 12/2012 |  |
| 2011/0048743 A1          | 3/2011           | Stafford et al.          | WO                                                                                                                                                                                                                                                                                                                                                                                               | 2013053057 A1 | 4/2013  |  |
| 2011/0056692 A1          | 3/2011           | Lopez de Cardenas et al. | WO                                                                                                                                                                                                                                                                                                                                                                                               | 2013078031 A1 | 5/2013  |  |
| 2011/0056702 A1          | 3/2011           | Sharma et al.            | OTHER PUBLICATIONS                                                                                                                                                                                                                                                                                                                                                                               |               |         |  |
| 2011/0067872 A1          | 3/2011           | Agrawal                  | International Search Report and Written Opinion; Mail Date Jul. 28, 2011; International Application No. PCT/US2010/057763; International Filing date Nov. 23, 2010; Korean Intellectual Property Office; International Search Report 7 pages; Written Opinion 3 pages.                                                                                                                           |               |         |  |
| 2011/0067889 A1          | 3/2011           | Marya et al.             | Flow Control Systems, [online]; [retrieved on May 20, 2010]; retrieved from the Internet <a href="http://www.bakerhughes.com/products-and-services/completions-and-productions/well-completions/packers-and-flow-control/flow-control-systems">http://www.bakerhughes.com/products-and-services/completions-and-productions/well-completions/packers-and-flow-control/flow-control-systems</a> . |               |         |  |
| 2011/0067890 A1          | 3/2011           | Themig                   | Optisleeve Sliding Sleeve, [online]; [retrieved on Jun. 25, 2010]; retrieved from the Internet <a href="http://weatherford.com/weatherford/groups/.../weatherfordcorp/WFT033159.pdf">weatherford.com/weatherford/groups/.../weatherfordcorp/WFT033159.pdf</a> .                                                                                                                                  |               |         |  |
| 2011/0094406 A1          | 4/2011           | Marya et al.             | “Sliding Sleeve”, Omega Completion Technology Ltd, Sep. 29, 2009, retrieved on: <a href="http://www.omega-completion.com">www.omega-completion.com</a> .                                                                                                                                                                                                                                         |               |         |  |
| 2011/0100643 A1          | 5/2011           | Themig et al.            | Welch, William R. et al., “Nonelastomeric Sliding Sleeve Maintains Long Term Integrity in HP/HT Application: Case Histories.” [Abstract Only], SPE Eastern Regional Meeting, Oct. 23-25, 1996, Columbus, Ohio.                                                                                                                                                                                   |               |         |  |
| 2011/0127044 A1          | 6/2011           | Radford et al.           | Ambat, et al.; “Electroless Nickel-Plating on AZ91D Magnesium Alloy: Effect of Substrate Microstructure and Plating Parameters”, Surface and Coatings Technology; 179; pp. 124-134; (2004).                                                                                                                                                                                                      |               |         |  |
| 2011/0132621 A1          | 6/2011           | Agrawal et al.           | Chang, et al.; “Electrodeposition of Aluminum on Magnesium Alloy in Aluminum Chloride (AlC13)-1-ethyl-3-methylimidazolium chloride (EMIC) Ionic Liquid and Its Corrosion Behavior”; Electrochemistry Communications; 9; pp. 1602-1606; (2007).                                                                                                                                                   |               |         |  |
| 2011/0139465 A1          | 6/2011           | Tibbles et al.           | Forsyth, et al.; “An Ionic Liquid Surface Treatment for Corrosion Protection of Magnesium Alloy AZ31”; Electrochem. Solid-State Lett./ 9(11); Abstract only; 1 page.                                                                                                                                                                                                                             |               |         |  |
| 2011/0147014 A1          | 6/2011           | Chen et al.              | Forsyth, et al.; “Exploring Corrosion Protection of Mg via Ionic Liquid Pretreatment”; Surface & Coatings Technology; 201; pp. 4496-4504; (2007).                                                                                                                                                                                                                                                |               |         |  |
| 2011/0186306 A1          | 8/2011           | Marya et al.             | Hsiao et al.; “Effect of Heat Treatment on Anodization and Electrochemical Behavior of AZ91D Magnesium Alloy”; J. Mater. Res.; 20(10); pp. 2763-2771; (2005).                                                                                                                                                                                                                                    |               |         |  |
| 2011/0214881 A1          | 9/2011           | Newton et al.            | Hsiao, et al.; “Anodization of AZ91D Magnesium Alloy in Silicate-Containing Electrolytes”; Surface & Coatings Technology; 199; pp. 127-134; (2005).                                                                                                                                                                                                                                              |               |         |  |
| 2011/0247833 A1          | 10/2011          | Todd et al.              | Hsiao, et al.; “Baking Treatment Effect on Materials Characteristics and Electrochemical Behavior of anodic Film Formed on AZ91D Magnesium Alloy”; Corrosion Science; 49; pp. 781-793; (2007).                                                                                                                                                                                                   |               |         |  |
| 2011/0253387 A1          | 10/2011          | Ervin                    | Hsiao, et al.; “Characterization of Anodic Films Formed on AZ91D Magnesium Alloy”; Surface & Coatings Technology; 190; pp. 299-308; (2005).                                                                                                                                                                                                                                                      |               |         |  |
| 2011/0256356 A1          | 10/2011          | Tomantschger et al.      | Huo et al.; “Corrosion of AZ91D Magnesium Alloy with a Chemical Conversion Coating and Electroless Nickel Layer”; Corrosion Science; 46; pp. 1467-1477; (2004).                                                                                                                                                                                                                                  |               |         |  |
| 2011/0259610 A1          | 10/2011          | Shkurti et al.           | Liu, et al.; “Electroless Nickel Plating on AZ91 Mg Alloy Substrate”; Surface & Coatings Technology; 200; pp. 5087-5093; (2006).                                                                                                                                                                                                                                                                 |               |         |  |
| 2011/0277987 A1          | 11/2011          | Frazier                  | Shi et al.; “Influence of the Beta Phase on the Corrosion Performance of Anodised Coatings on Magnesium—Aluminium Alloys”; Corrosion Science; 47; pp. 2760-2777; (2005).                                                                                                                                                                                                                         |               |         |  |
| 2011/0277989 A1          | 11/2011          | Frazier                  | Song, et al.; “Corrosion Mechanisms of Magnesium Alloys”; Advanced Engineering Materials; 1(1); pp. 11-33; (1999).                                                                                                                                                                                                                                                                               |               |         |  |
| 2011/0284232 A1          | 11/2011          | Huang                    | Song, Guangling; “Recent Progress in Corrosion and Protection of Magnesium Alloys”; Advanced Engineering Materials; 7(7); pp. 563-586; (2005).                                                                                                                                                                                                                                                   |               |         |  |
| 2011/0284240 A1          | 11/2011          | Chen et al.              | Song, et al.; “Influence of Microstructure on the Corrosion of Diecast AZ91D”; Corrosion Science; 41; pp. 249-273; (1999).                                                                                                                                                                                                                                                                       |               |         |  |
| 2011/0284243 A1          | 11/2011          | Frazier                  | Song, et al.; “Corrosion Behaviour of AZ21, AZ501 and AZ91 in Sodium Chloride”; Corrosion Science; 40(10); pp. 1769-1791; (1998).                                                                                                                                                                                                                                                                |               |         |  |
| 2011/0300403 A1          | 12/2011          | Vecchio et al.           |                                                                                                                                                                                                                                                                                                                                                                                                  |               |         |  |
| 2012/0067426 A1          | 3/2012           | Soni et al.              |                                                                                                                                                                                                                                                                                                                                                                                                  |               |         |  |
| 2012/0103135 A1          | 5/2012           | Xu et al.                |                                                                                                                                                                                                                                                                                                                                                                                                  |               |         |  |
| 2012/0107590 A1          | 5/2012           | Xu et al.                |                                                                                                                                                                                                                                                                                                                                                                                                  |               |         |  |
| 2012/0118583 A1          | 5/2012           | Johnson et al.           |                                                                                                                                                                                                                                                                                                                                                                                                  |               |         |  |
| 2012/0130470 A1          | 5/2012           | Agnew et al.             |                                                                                                                                                                                                                                                                                                                                                                                                  |               |         |  |
| 2012/0145389 A1          | 6/2012           | Fitzpatrick, Jr.         |                                                                                                                                                                                                                                                                                                                                                                                                  |               |         |  |
| 2012/0168152 A1          | 7/2012           | Casciaro                 |                                                                                                                                                                                                                                                                                                                                                                                                  |               |         |  |
| 2012/0211239 A1          | 8/2012           | Kritzler et al.          |                                                                                                                                                                                                                                                                                                                                                                                                  |               |         |  |
| 2012/0267101 A1          | 10/2012          | Cooke                    |                                                                                                                                                                                                                                                                                                                                                                                                  |               |         |  |
| 2012/0292053 A1          | 11/2012          | Xu et al.                |                                                                                                                                                                                                                                                                                                                                                                                                  |               |         |  |
| 2012/0318513 A1          | 12/2012          | Mazyar et al.            |                                                                                                                                                                                                                                                                                                                                                                                                  |               |         |  |
| 2013/0004847 A1          | 1/2013           | Kumar et al.             |                                                                                                                                                                                                                                                                                                                                                                                                  |               |         |  |
| 2013/0025409 A1          | 1/2013           | Xu                       |                                                                                                                                                                                                                                                                                                                                                                                                  |               |         |  |
| 2013/0032357 A1          | 2/2013           | Mazyar et al.            |                                                                                                                                                                                                                                                                                                                                                                                                  |               |         |  |
| 2013/0048304 A1          | 2/2013           | Agrawal et al.           |                                                                                                                                                                                                                                                                                                                                                                                                  |               |         |  |
| 2013/0052472 A1          | 2/2013           | Xu                       |                                                                                                                                                                                                                                                                                                                                                                                                  |               |         |  |
| 2013/0081814 A1          | 4/2013           | Gaudette et al.          |                                                                                                                                                                                                                                                                                                                                                                                                  |               |         |  |
| 2013/0105159 A1          | 5/2013           | Alvarez                  |                                                                                                                                                                                                                                                                                                                                                                                                  |               |         |  |
| 2013/0126190 A1          | 5/2013           | Mazyar et al.            |                                                                                                                                                                                                                                                                                                                                                                                                  |               |         |  |
| 2013/0133897 A1          | 5/2013           | Baihly et al.            |                                                                                                                                                                                                                                                                                                                                                                                                  |               |         |  |
| 2013/0146144 A1          | 6/2013           | Joseph et al.            |                                                                                                                                                                                                                                                                                                                                                                                                  |               |         |  |
| 2013/0146302 A1          | 6/2013           | Gaudette et al.          |                                                                                                                                                                                                                                                                                                                                                                                                  |               |         |  |
| 2013/0186626 A1          | 7/2013           | Aitken et al.            |                                                                                                                                                                                                                                                                                                                                                                                                  |               |         |  |
| 2013/0240203 A1          | 9/2013           | Frazier                  |                                                                                                                                                                                                                                                                                                                                                                                                  |               |         |  |
| 2013/0327540 A1          | 12/2013          | Hamid et al.             |                                                                                                                                                                                                                                                                                                                                                                                                  |               |         |  |
| 2014/0116711 A1          | 5/2014           | Tang et al.              |                                                                                                                                                                                                                                                                                                                                                                                                  |               |         |  |
| FOREIGN PATENT DOCUMENTS |                  |                          |                                                                                                                                                                                                                                                                                                                                                                                                  |               |         |  |
| CN                       | 101050417 A      | 10/2007                  |                                                                                                                                                                                                                                                                                                                                                                                                  |               |         |  |
| CN                       | 101351523 A      | 1/2009                   |                                                                                                                                                                                                                                                                                                                                                                                                  |               |         |  |
| CN                       | 101457321 B      | 6/2009                   |                                                                                                                                                                                                                                                                                                                                                                                                  |               |         |  |
| EP                       | 0033625 A1       | 8/1981                   |                                                                                                                                                                                                                                                                                                                                                                                                  |               |         |  |
| EP                       | 1857570 A2       | 11/2007                  |                                                                                                                                                                                                                                                                                                                                                                                                  |               |         |  |
| GB                       | 912956           | 12/1962                  |                                                                                                                                                                                                                                                                                                                                                                                                  |               |         |  |
| JP                       | 61067770         | 4/1986                   |                                                                                                                                                                                                                                                                                                                                                                                                  |               |         |  |
| JP                       | 7-54008          | 2/1995                   |                                                                                                                                                                                                                                                                                                                                                                                                  |               |         |  |
| JP                       | 08232029         | 9/1996                   |                                                                                                                                                                                                                                                                                                                                                                                                  |               |         |  |
| JP                       | 08-232029 A1     | 10/1996                  |                                                                                                                                                                                                                                                                                                                                                                                                  |               |         |  |
| JP                       | 2010502840 A     | 1/2010                   |                                                                                                                                                                                                                                                                                                                                                                                                  |               |         |  |
| KR                       | 95-0014350 B1    | 11/1995                  |                                                                                                                                                                                                                                                                                                                                                                                                  |               |         |  |

(56)

## References Cited

## OTHER PUBLICATIONS

- Zhang, et al; "Study on the Environmentally Friendly Anodizing of AZ91D Magnesium Alloy"; Surface and Coatings Technology: 161; pp. 36-43; (2002).
- H. Watarai, Trend of research and development for magnesium alloys—reducing the weight of structural materials in motor vehicles, (2006) Science and technology trends, Quaterly review No. 18, 84-97.
- M. Bououdina, Z. X. Guo, Comparative study of mechanical alloying of (Mg+Al) and (Mg+Al+Ni) mixtures for hydrogen storage, *J. Alloys, Compds.* 2002, 336, 222-231.
- M.Liu, P.J. Uggowitzer, A.V. Nagasekhar, P. Schmutz, M. Easton, G.L. Song, A. Atrens, Calculated phase diagrams and the corrosion of die-cast Mg—Al alloys, *Corrosion Science*, 2009, 51, 606-619.
- S.L. Lee, C.W. Hsu, F.K. Hsu, C.Y. Chou, C.K. Lin, C.W. Weng, Effects of Ni addition on hydrogen storage properties of Mg17Al12alloy, *Materials Chemistry and Physics*, 2011, 126, 319-324.
- T.J. Bastow, S. Celotto, Clustering and formation of nano-precipitates in dilute aluminum and magnesium alloys, *Materials science and Engineering*, 2003, C23, 757-762.
- Canadian Pat. App. No. 2783241 filed on Dec. 7, 2010 titled Nanomatrix Powder Metal Compact.
- Canadian Pat. App. No. 2783346 filed on Dec. 7, 2010, published on Jun. 16, 2011 for "Engineered Powder Compact Composite Material".
- Pardo, et al.; "Corrosion Behaviour of Magnesium/Aluminium Alloys in 3.5 wt% NaCl"; *Corrosion Science*; 50; pp. 823-834; (2008).
- Song, et al.; "Understanding Magnesium Corrosion"; *Advanced Engineering Materials*; 5; No. 12; pp. 837-858; (2003).
- Chun-Lin, Li. "Design of Abrasive Water Jet Perforation and Hydraulic Fracturing Tool," *Oil Field Equipment*, Mar. 2011.
- M. Toyoda et al., "Sorption and recovery of heavy oil by using exfoliated graphite," *Desalination* 115 (1998), pp. 199-201.
- T. Enoki et al., "Exfoliated Graphite Formed by Intercalation," *Graphite Intercalation Compounds and Applications*, Copyright © 2003 by Oxford University Press, Inc., pp. 403-413.
- T. Masahiro et al., "Heavy oil sorption using exfoliated graphite New application of exfoliated graphite to protect heavy oil pollution," *Carbon* 38 (2000), pp. 199-210.
- V. Smuleac et al., "Polythiol-functionalized alumina membranes for mercury capture," *Journal of Membrane Sciences* 251 (2005), pp. 169-178.
- W. Gao et al., "Engineered Graphite Oxide Materials for Application in Water Purification," *ACS Appl. Mater. Interfaces* 2011, 3, pp. 1821-1826.
- Yadira I. Vega-Cantu, "Studies on Nitrile Rubber Degradation in Zinc Bromide Completion Fluid and its Prevention by Surface Fluorination," *Rice University, Houston Texas, Sep. 2001*, 138p.
- Constantine, Jesse. "Selective Production of Horizontal Openhole Completions Using ECP and Sliding Sleeve Technology." *SPE Rocky Mountain Regional Meeting*, May 15-18, 1999, Gillette, Wyoming. [Abstract Only].
- Elsayed Ayman, Imai Hisashi, Umeda Junko and Kondoh Katsuyoshi, "Effect of Consolidation and Extrusion Temperatures on Tensile Properties of Hot Extruded ZK61 Magnesium Alloy Gas Atomized Powders via Spark Plasma Sintering" *Transacation of JWRI*, vol. 38, (2009) No. 2, pp. 31-35.
- Forsyth, et al.; "An Ionic Liquid Surface Treatment for Corrosion Protection of Magnesium Alloy AZ31"; *Electrochem. Solid-State Lett.* 9(11); Abstract only; Aug. 29, 2006; 1 page.
- Bing Q. Han, Enrique J. Lavernia and Farghali A. Mohamed, "Mechanical Properties of Nanostructured Materials", *Rev. Adv. Mater. Sci.* 9(2005) 1-16.
- International Search Report and Written Opinion for PCT Application No. PCT/US2012/044866, dated Jan. 2, 2013, pp. 1-9.
- International Search Report and Written Opinion, PCT/US2012/046231, Date of Mailing Jan. 29, 2013, Korean Intellectual Property Office, Written Opinion 6 pages, International Search Report 3 pages.
- Lunder et al.; "The Role of Mg17Al12 Phase in the Corrosion of Mg Alloy AZ91"; *Corrosion*; 45(9); pp. 741-748; (1989).
- Adam J. Maisano, "Cryomilling of Aluminum-Based and Magnesium-Based Metal Powders", Thesis, Virginia Tech, Jan. 13, 2006.
- Nie, Xiaowu. "Patents of Methods to Prepare Intermetallic Matrix Composites: A Review," *Recent Patents on Materials Science* 2008, vol. 1, pp. 232-240.
- International Search Report and Written Opinion, International Application No. PCT/US2012/049434, Date of Mailing Feb. 1, 2013, Korean Intellectual Property Office, Written Opinion 4 pages, International Search Report 3 pages.
- E.J. Lavenia, B.Q. Han, J.M. Schoenung: "Cryomilled nanostructured materials: Processing and properties", *Materials Science and Engineering A*, 493, (2008) 207-214.
- International Search Report and Written Opinion; International Application No. PCT/US2012/038622; International Filing Date: May 18, 2012; Date of Mailing Dec. 6, 2012; 12 pages.
- International Search Report and Written Opinion; International Application No. PCT/US2010/057763; International Filing date Nov. 23, 2010; Korean Intellectual Property Office; International Search Report 7 pages; Written Opinion 3 pages, Jul. 28, 2011.
- International Search Report and Written Opinion; PCT/US2010/059257; Korean Intellectual Property Office; dated Jul. 27, 2011.
- Notification of Transmittal of the International Search Report and the Written Opinion of the International Searching Authority; PCT/US2010/059259; International Searching Authority KIPO; Mailed Jun. 13, 2011.
- International Search Report and Written Opinion, PCT/US2010/059263, dated Jul. 8, 2011.
- Notification of Transmittal of the International Search Report and the Written Opinion of the International Searching Authority; PCT/US2010/059265; International Searching Authority KIPO; Mailed Jun. 16, 2011.
- Notification of Transmittal of the International Search Report and the Written Opinion of the International Searching Authority; PCT/US2010/059268; International Searching Authority KIPO; Mailed Jun. 17, 2011.
- Notification of Transmittal of the International Search Report and the Written Opinion of the International Searching Authority, or the Declaration mailed on Feb. 23, 2012 (Dated Feb. 22, 2012) for PCT/US2011/043036.
- Notification of Transmittal of the International Search Report and the Written Opinion of the International Searching Authority; PCT/US2011/047000; Korean Intellectual Property Office; Mailed Dec. 26, 2011; 8 pages.
- International Search Report and Written Opinion of the International Searching Authority for International Application No. PCT/US2011/058099 (filed on Oct. 27, 2011), mailed on May 11, 2012.
- International Search Report and Written Opinion of the International Searching Authority, or the Declaration for PCT/US2011/058105 mailed from the Korean Intellectual Property Office on May 1, 2012.
- International Search Report and Written Opinion for International application No. PCT/US2012/034973 filed on Apr. 25, 2012, mailed on Nov. 29, 2012.
- Patent Cooperation Treaty International Search Report and Written Opinion for International Patent Application No. PCT/US2012/034978 filed on Apr. 25, 2012, mailed on Nov. 12, 2012.
- International Search Report and Written Opinion; PCT/US2012/038622; Dated Dec. 6, 2012; 12 pages.
- Shumbera et al. "Improved Water Injector Performance in a Gulf of Mexico Deepwater Development Using an Openhole Frac Pack Completion and Downhole Filter System: Case History." *SPE Annual Technical Conference and Exhibition*, Oct. 5-8, 2003, Denver, Colorado. [Abstract Only].
- Vickery, Harold and Christian Bayne, "New One-Trip Multi-Zone Frac Pack System with Positive Positioning." *European Petroleum Conference*, Oct. 29-31, 2002, Aberdeen, UK. [Abstract Only].
- H. Watanabe, T. Mukai, M. Mabuchi and K. Higashi, "Superplastic Deformation Mechanism in Powder Metallurgy Magnesium Alloys and Composites", *Acta mater.* 49 (2001) pp. 2027-2037.
- Xiaowu Nie, Patents of Methods to Prepare Intermetallic Matrix Composites: A Review, *Recent Patents on Materials Science* 2008, 1,

(56)

## References Cited

## OTHER PUBLICATIONS

- 232-240, Department of Scientific Research, Hunan Railway College of Science and Technology, Zhuzhou, P.R. China.
- Baker Oil Tools. "Z-Seal Metal-to-Metal Expandable Sealing Device Uses Expanding Metal in Place of Elastomers," Nov. 6, 2006.
- C.S. Goh, J. Wei, L C Lee, and M. Gupta, "Development of novel carbon nanotube reinforced magnesium nanocomposites using the powder metallurgy technique", *Nanotechnology* 17 (2006) 7-12.
- CH. Christoglou, N. Voudouris, G.N. Angelopoulos, M. Pant, W. Dahl, "Deposition of Aluminum on Magnesium by a CVD Process", *Surface and Coatings Technology* 184 (2004) 149-155.
- Chinese Office Action for related CN Application No. 201180052095.6, dated Jul. 21, 2014, pp. 1-32.
- E. Paul Bercegeay et al., "A One-Trip Gravel Packing System"; Society of Petroleum Engineers, Offshore Technology Conference, SPE Paper No. 4771; Feb. 7-8, 1974.
- Hjortstam et al. "Can we achieve ultra-low resistivity in carbon nanotube-based metal composites," *Applied Physics A* (2004), vol. 78, Issue 8, pp. 1175-1179. [Abstract Only].
- J. Dutta Majumdar, B. Ramesh Chandra, B.L. Mordike, R. Galun, I. Manna, "Laser Surface Engineering of a Magnesium Alloy with Al+Al<sub>2</sub>O<sub>3</sub>", *Surface and Coatings Technology* 179 (2004) 297-305.
- Shimizu et al., "Multi-walled carbon nanotube-reinforced magnesium alloy composites", *Scripta Materialia*, vol. 58, Issue 4, pp. 1-13.
- Song, G. and S. Song. "A Possible Biodegradable Magnesium Implant Material," *Advanced Engineering Materials*, vol. 9, Issue 4, Apr. 2007, pp. 298-302. [Abstract Only].
- Wikipedia, the free encyclopedia. Reactivity series. [http://en.wikipedia.org/w/index.php?title=Reactivity\\_series&printable=yes](http://en.wikipedia.org/w/index.php?title=Reactivity_series&printable=yes) downloaded on May 18, 2014. 8 pages.
- Xiaotong Wang et al., "Contact-Damage-Resistant Ceramic/Single-Wall Carbon Nanotubes and Ceramic/Graphite Composites" *Nature Materials*, vol. 3, Aug. 2004, pp. 539-544.
- Y. Zhang and Hongjie Dai, "Formation of metal nanowires on suspended single-walled carbon nanotubes" *Applied Physics Letter*, vol. 77, No. 19 (2000), pp. 3015-3017.
- Y. Zhang, Nathan W. Franklin, Robert J. Chen, Hongjie Dai, "Metal Coating on Suspended Carbon Nanotubes and its Implication to Metal—Tube Interaction", *Chemical Physics Letters* 331 (2000) 35-41.
- Zeng et al. "Progress and Challenge for Magnesium Alloys as Biomaterials," *Advanced Engineering Materials*, vol. 10, Issue 8, Aug. 2008, pp. B3-B14. [Abstract Only].
- Adams, et al., "Thermal stabilities of aromatic acids as geothermal tracers", *Geothermics*, vol. 21, No. 3, 1992, pp. 323-339.
- Ayman, et al.; "Effect of Consolidation and Extrusion Temperatures on Tensile Properties of Hot Extruded ZK61 Magnesium Alloy Gas Atomized Powders via Spark Plasma Sintering", *Transactions of JWRI*, vol. 38 (2009), No. 2, pp. 1-5.
- Canadian Office Action for Canadian Application No. 2,783,547, dated Feb. 15, 2013, pp. 1-3.
- Canadian Office Action for Canadian Application No. 2,833,958, dated Sep. 23, 2014, pp. 1-2.
- Carrejo, et al., "Improving Flow Assurance in Multi-Zone Fracturing Treatments in Hydrocarbon Reservoirs with High Strength Corrodible Tripping Balls"; Society of Petroleum Engineers; SPE Paper No. 151613; Apr. 16, 2012; 6 pages.
- Chinese Office Action for Chinese Application No. 201080055613.5, dated Nov. 4, 2014, pp. 1-20.
- Feng, et al., "Electroless Plating of Carbon Nanotubes with Silver" *Journal of Materials Science*, 39, (2004) pp. 3241-3243.
- Garfield, New One-Trip Sand-Control Completion System that Eliminates Formation Damage Resulting From conventional Perforating and Gravel-Pack Operations:, SPE Annual Technical Conference and Exhibition, Oct. 9-12, 2005.
- Garfield, et al., "Maximizing Inflow Performance in Soft Sand Completions Using New One-trip Sand Control Liner Completion Technology", SPE European Formation Damage Conference, May 25-27, 2005.
- International Search Report and Written Opinion; International Application No. PCT/US2012/053339; International Filing Date: Aug. 31, 2012; Date of Mailing: Feb. 15, 2013; 11 pages.
- International Search Report and Written Opinion; International Application No. PCT/US2012/053342; International Filing Date: Aug. 31, 2012; Date of Mailing: Feb. 19, 2013; 9 pages.
- International Search Report and Written Opinion; International Application No. PCT/US2012/053350; International Filing Date: Aug. 31, 2012; Date of Mailing: Feb. 25, 2013; 10 pages.
- International Search Report and Written Opinion; International Application No. PCT/US2014/049347; International Filing Date: Aug. 1, 2014; Date of Mailing: Nov. 24, 2014; 11 pages.
- International Search Report and Written Opinion; International Application No. PCT/US2014/054720; International Filing Date: Sep. 9, 2014; Date of Mailing: Dec. 17, 2014; 10 pages.
- Li, et al., "Investigation of aluminium-based nanocomposites with ultra-high strength", *Materials Science and Engineering A*, 527, pp. 305-316. (2009).
- Mathis, "Sand Management: A Review of Approaches and Concerns", Society of Petroleum Engineers, SPE Paper No. 82240, SPE European Formation Damage Conference, The Hague, The Netherlands, May 13-14, 2003.
- Rose, et al.; "The application of the polycyclic aromatic sulfonates as tracers in geothermal reservoirs", *Geothermics* 30 (2001) pp. 617-640.
- Seyni, et al., "On the interest of using degradable fillers in co-ground composite materials", *Powder Technology* 190, (2009) pp. 176-184.
- Shaw, "Benefits and Application of a Surface-Controlled Sliding Sleeve for Fracturing Operations"; Society of Petroleum Engineers, SPE Paper No. 147546; Oct. 30, 2011; 8 pages.
- Shigematsu, et al., "Surface Treatment of AZ91D Magnesium Alloy by Aluminum diffusion Coating", *Journal of Materials Science Letters* 19, 2000, pp. 473-475.
- Singh, et al., "Extended Homogeneity Range of Intermetallic Phases in Mechanically Alloyed Mg—Al Alloys", Elsevier Sciences Ltd., *Intermetallics* 11, 2003, pp. 373-376.
- Stanley, et al.; "An Introduction to Ground-Water Tracers", Department of Hydrology and Water Resources, University of Arizona, Mar. 1985, pp. 1-219.
- Walters, et al.; "A Study of Jets from Unsintered-Powder Metal Lined Nonprecision Small-Caliber Shaped Charges", Army Research Laboratory, Aberdeen Proving Ground, MD 21005-5066; Feb. 2001.
- Xu, et al., "Nanostructured Material-Based Completion Tools Enhance Well Productivity"; International Petroleum Technology Conference; Conference Paper IPTC 16538; International Petroleum Technology Conference 2013; 4 pages.
- Zemel, "Tracers in the Oil Field", University of Texas at Austin, Center for Petroleum and Geosystems, Jan. 1995, Chapters 1, 2, 3, 7.
- Zhang, et al.; "High Strength Nanostructured Materials and Their Oil Field Applications"; Society of Petroleum Engineers; Conference Paper SPE 157092; SPE International Oilfield Nanotechnology Conference, 2012; 6 pages.
- Canadian Office Action for Canadian Application No. 2,834,794, dated Dec. 15, 2014, pp. 1-3.
- Danish Search Report and Opinion for Danish Application No. PA 2013 00060, dated Dec. 12, 2014, pp. 1-6.
- International Search Report and Written Opinion; International Application No. PCT/US2012/071742; International Filing Date: Dec. 27, 2012; Date of Mailing: Apr. 22, 2013; 12 pages.
- International Search Report and Written Opinion; International Application No. PCT/US2014/058997, International Filing Date: Oct. 3, 2014; Date of Mailing: Jan. 12, 2015; 12 pages.
- International Search Report; International Application No. PCT/US2012/044229, International Filing Date: Jun. 26, 2012; Date of Mailing: Jan. 30, 2013; 3 pages.
- Murray, "Binary Alloy Phase Diagrams" *Int. Met. Rev.*, 30(5) 1985 vol. 1, pp. 103-187.
- Vernon Constien et al., "Development of Reactive Coatings to Protect Sand-Control Screens", SPE 112494, Copyright 2008, Society of Petroleum Engineers, Presented at the 2008 SPE International Symposium and Exhibition on Formation Damage Control.

FIG. 1



FIG. 2A



FIG. 2B



FIG. 2C



## 1

**CORRODIBLE DOWNHOLE ARTICLE AND  
METHOD OF REMOVING THE ARTICLE  
FROM DOWNHOLE ENVIRONMENT**

BACKGROUND

Certain downhole operations involve placement of elements in a downhole environment, where the element performs its function, and is then removed. For example, elements such as ball/ball seat assemblies and fracture (frac) plugs are downhole elements used to seal off lower zones in a borehole in order to carry out a hydraulic fracturing process (also referred to in the art as "fracking") to break up reservoir rock. After the fracking operation, the ball/ball seat or plugs are then removed to allow fluid flow to or from the fractured rock.

To facilitate removal, such elements may be formed of a material that reacts with the ambient downhole environment so that they need not be physically removed by, for example, a mechanical operation, but may instead corrode or dissolve under downhole conditions. However, because operations such as fracking may not be undertaken for months after the borehole is drilled, such elements may have to be immersed in downhole fluids for extended periods of time (for example, up to a year, or longer) before the fracking operation begins. Therefore, it is desirable to have corrodible downhole elements such as ball seats and frac plugs that are protected from uncontrolled corrosion during that period of time, and which then can be subsequently made corrodible as needed.

SUMMARY

The above and other deficiencies of the prior art are overcome by a method of removing a corrodible downhole article having a surface coating, comprising eroding the surface coating by physical abrasion, chemical etching, or a combination of physical abrasion and chemical etching, the surface coating comprising a metallic layer of a metal resistant to corrosion by a corrosive material.

In another embodiment, a method of removing a corrodible downhole article which comprises a magnesium alloy core, and a metallic layer covering the magnesium alloy core, the metallic layer being resistant to corrosion by a corrosive material, the method comprising eroding the metallic layer by physical abrasion, chemical etching, or a combination of physical abrasion and chemical etching, and corroding the corrodible downhole article in a corrosive material after eroding.

In another embodiment, an article for forming a downhole seal comprises a magnesium alloy core, and a metallic layer having a thickness of about 100 to about 500 micrometers and covering the magnesium alloy core, the metallic layer being formed of nickel, aluminum, or an alloy thereof, and resistant to corrosion by a corrosive material, the article being a ball seat or frac plug.

In another embodiment, a method of making an article for forming a downhole seal, comprising plating, in the absence of water, a metallic layer having a thickness of about 100 to about 500 micrometers and resistant to corrosion by a corrosive material, on a surface of a magnesium alloy core, the article being a ball seat or frac plug.

BRIEF DESCRIPTION OF THE DRAWINGS

Referring now to the drawings wherein like elements are numbered alike in the several Figures:

## 2

FIG. 1 shows a cross-sectional view of a corrodible downhole article 100 prior to removal of a protective coating 111 and seating of a ball 130; and

FIGS. 2A-2C show cross-sectional views of the sequential process for removing a protective coating 211 from a corrodible downhole article 200 (FIG. 2A), seating a ball 230 (FIG. 2B) in a seating zone 210 before fracking, and removing the ball 230 and seating zone 210 after fracking (FIG. 2C).

10 DETAILED DESCRIPTION OF THE INVENTION

A corrodible downhole article is disclosed, such as a ball seat or frac plug, where the downhole article includes a corrodible core, which dissolves in a corrosive environment, and a metallic layer covering the core. The metallic layer has sufficient thickness to resist scratching and premature erosion, but which is thin enough to be eroded physically, chemically, or by a combination including at least one of these types of processes prior to seating a ball on the ball seat. In this way, the seated core can be exposed to the corrosive downhole environment and the corrodible core corroded away to remove the article.

The corrodible downhole article, which is useful for forming a seal, includes a corrodible core that corrodes under downhole conditions, and a surface coating, which includes a metallic layer. The corrodible core has the surface coating on a surface of the core material.

The corrodible core comprises any material suitable for use in a downhole environment provided the core material is 25 corrodible in the downhole environment. Core materials can include corrodible metals, metal oxides, composites, soluble glasses, and the like. Useful such core materials dissolve 30 under aqueous conditions.

In an embodiment, the core material is a magnesium alloy. 35 The magnesium alloy core includes magnesium or any magnesium alloy which is dissolvable in a corrosive environment including those typically encountered downhole, such as an aqueous environment which includes salt (i.e., brine), or an acidic or corrosive agent such as hydrogen sulfide, hydrochloric acid, or other such corrosive agents. Magnesium 40 alloys suitable for use include alloys of magnesium with aluminum (Al), cadmium (Cd), calcium (Ca), cobalt (Co), copper (Cu), iron (Fe), manganese (Mn), nickel (Ni), silicon (Si), silver (Ag), strontium (Sr), thorium (Th), tungsten (W), 45 zinc (Zn), zirconium (Zr), or a combination comprising at least one of these elements. Particularly useful alloys include magnesium alloy particles including those prepared from magnesium alloyed with Ni, W, Co, Cu, Fe, or other metals. Alloying or trace elements can be included in varying 50 amounts to adjust the corrosion rate of the magnesium. For example, four of these elements (cadmium, calcium, silver, and zinc) have to mild-to-moderate accelerating effects on corrosion rates, whereas four others (copper, cobalt, iron, and nickel) have a still greater effect on corrosion. Exemplary 55 commercial magnesium alloys which include different combinations of the above alloying elements to achieve different degrees of corrosion resistance include but are not limited to, for example, those alloyed with aluminum, strontium, and manganese such as AJ62, AJ50x, AJ51x, and AJ52x alloys, and those alloyed with aluminum, zinc, and manganese such as AZ91A-E alloys.

It will be appreciated that alloys having corrosion rates greater than those of the above exemplary alloys are contemplated as being useful herein. For example, nickel has been 60 found to be useful in decreasing the corrosion resistance (i.e., increasing the corrosion rate) of magnesium alloys when included in small amounts (i.e., less than 1% by weight). In an

embodiment, the nickel content of a magnesium alloy is less than or equal to about 0.5 wt %, specifically less than or equal to about 0.4 wt %, and more specifically less than or equal to about 0.3 wt %, to provide a useful corrosion rate for the corrodible downhole article. In an exemplary embodiment, the magnesium particles are alloyed with about 0.25 wt % Ni.

The above magnesium alloys are useful for forming the core, and are formed into the desired shape and size by casting, forging and machining. Alternatively, powders of magnesium or the magnesium alloy are useful for forming the core. The magnesium alloy powder generally has a particle size of from about 50 to about 150 micrometers ( $\mu\text{m}$ ), and more specifically about 60 to about 140  $\mu\text{m}$ . The powder is further coated using a method such as chemical vapor deposition, anodization or the like, or admixed by physical method such cryo-milling, ball milling, or the like, with a metal or metal oxide such as Al, Ni, W, Co, Cu, Fe, oxides of one of these metals, or the like. Such coated magnesium powders are referred to herein as controlled electrolytic materials (CEM). The CEM materials are then molded or compressed into the desired shape by, for example, cold compression using an isostatic press at about 40 to about 80 ksi (about 275 to about 550 MPa), followed by forging or sintering and machining, to provide a core having the desired shape and dimensions.

It will be understood that the magnesium alloys, including CEM materials, will thus have any corrosion rate necessary to achieve the desired performance of the article. In a specific embodiment, the magnesium alloy or CEM material used to form the core has a corrosion rate of about 0.1 to about 20 mg/cm<sup>2</sup>/hour, specifically about 1 to about 15 mg/cm<sup>2</sup>/hour determined in aqueous 3 wt % KCl solution at 200° F. (93° C.).

The corrodible downhole article further has a surface coating, which includes a metallic layer. The metallic layer is resistant to corrosion by a corrosive material. As used herein, "resistant" means the metallic layer is not etched or dissolved by any corrosive downhole conditions encountered (i.e., brine, hydrogen sulfide, etc., at pressures greater than atmospheric pressure, and at temperatures in excess of 50° C.) such that any portion of the magnesium alloy core is exposed, for a period of greater than or equal to one year, specifically for a period of greater than or equal to two years.

The metallic layer includes any metal resistant to corrosion under ambient downhole conditions, and which can be removed by eroding as explained below. In an embodiment, the metallic layer includes nickel, aluminum, alloys thereof, or a combination comprising at least one of the foregoing. In an embodiment, the metallic layer is aluminum or aluminum alloy. In an embodiment, the metallic layer includes a single layer, or includes multiple layers of the same or different metals. In this way, the surface coating includes, in an embodiment, a metallic layer disposed on the core, and one or more additional layers of metal and/or metal oxide on the metallic layer. In an embodiment, adjacent, contacting layers in the surface coating have different compositions (e.g., are of different metals, combinations of metal and metal oxide, etc.). Such outer layers may be formed by coating the metal layer with another metal, forming an oxide or anodized layer, or any such method of forming the outer layers.

The metallic layer has a thickness of less than or equal to about 1,000 micrometers (i.e., about 1 millimeter). In an embodiment, the metallic layer may have a thickness of about 10 to about 1,000 micrometers, specifically about 50 to about 750 micrometers and still more specifically about 100 to about 500 micrometers. The metallic layer covers a portion of the surface of the magnesium alloy core, or covers the entirety of the magnesium alloy core.

The metallic layer is applied to the corrodible core by any suitable method, provided that the application process is not carried out in the presence of agents which can react with the magnesium core, and which cause damage to the surface of the magnesium metal core, such that the desired properties of the metallic layer or magnesium alloy core are substantially adversely affected.

The metallic layer is thus formed by any suitable method for depositing a metal, including an electroless plating process, or by electrodeposition. Any suitable known method for applying the metallic layer can be used, provided the method does not significantly adversely affect the performance of the core after plating, such as by non-uniform plating or formation of surface defects affecting the integrity of the plated metallic layer on the magnesium alloy core.

Electroless deposition is useful for applying a uniform layer of metal over complex surface geometries. For example, the metal coating can be a nickel coating applied by an electroless process to the magnesium core such as that described by Ambat et al. (Rajan Ambat, W. Zhou, *Surf. And Coat. Technol.* 2004, vol. 179, pp. 124-134) or by Liu et al. (Zhenmin Liu, Wei Gao, *Surf. And Coat. Technol.* 2006, vol. 200, pp. 5087-93), the contents of both of which are incorporated herein by reference in their entirety.

In another embodiment, plating is carried out by electrodeposition in the presence of an anhydrous ionic solvent (i.e., in the absence of moisture). It will be appreciated that the presence of adventitious water during the plating process may cause surface pitting, or may cause formation of metal hydroxides, such as magnesium hydroxide, on the surface of the magnesium alloy core. Such surface defects may lead to a non-uniform adhesion of the metallic layer to the core, or may undesirably cause surface defects which can lead to weakened or compromised integrity of the metallic layer, hence reducing the effectiveness of the metallic layer in protecting the magnesium alloy core against corrosion.

A useful method of making an article thus includes plating the metallic layer in the absence of water, to form a metallic layer having a thickness of about 100 to about 500 micrometers and resistant to corrosion by a corrosive material, on a surface of a magnesium alloy core. For example, electrodeposition to apply an aluminum coating on a surface of a magnesium alloy can be carried out using, as a plating medium, aluminum chloride in 1-ethyl-3-methylimidazolium chloride as an ionic liquid, according to the literature method of Chang et al. (Jeng-Kuei Chang, Su-Yau Chen, Wen-Ta Tsai, Ming-Jay Deng, I-Wen Sun, *Electrochem. Comm.* 2007, vol. 9, pp. 1602-6), the contents of which are incorporated herein by reference in their entirety. In an embodiment, the article is a ball seat or frac plug.

Articles useful for downhole applications include ball seats and frac plugs. In an embodiment, the article has a generally cylindrical shape that tapers in a truncated, conical cross-sectional shape such as a ball seat, with an inside diameter in cylindrical cross-section of about 2 to about 15 cm, sufficient to allow, for example, a ball to fit downhole and to seat and form a seal in the desired downhole element. In a further embodiment, the surface is milled to have a concave region having a radius designed to accommodate a ball or plug.

In an embodiment, a method of removing the corrodible downhole article from a downhole environment includes eroding the surface coating of the article by physical abrasion, chemical etching, or a combination of physical abrasion and chemical etching, the surface coating being a metallic layer of a metal resistant to corrosion by a corrosive material. In another embodiment, the eroding is accomplished by physical abrasion alone.

Eroding comprises flowing a slurry of a proppant over the surface of the corrodible downhole article. A proppant includes any material useful for injecting into the fractured zones after the fracking process, to prop open the fractures in the downhole rock. Proppants useful herein have a hardness and abrasiveness greater than that of the surface layer. For example, useful proppants include sand including rounded sand grains, aluminum pellets, glass beads, ceramic beads including those based on alumina and zirconia, and the like, and combinations comprising at least one of the foregoing. In some embodiments, the proppant is polymer coated or is coated with a curable resin. Typical proppants have a mesh size of about 12 to about 70 mesh. The proppant is slurried in any suitable fluid used for fracking or other downhole fluid. For example, the fracking fluid includes distillate, diesel fuel, kerosene, polymer-based fluids, and aqueous fluids such as water, brine, dilute hydrochloric acid, or aqueous viscoelastic fluids such as those described in U.S. Pat. No. 7,723,272 which contains water, a viscoelastic surfactant (VES), additives to reduce viscosity (after delivery of the proppant), viscosity stabilizers and enhancers, and fluid loss control agents. A mixture of these fracking fluids with other solvents and/or surfactants commonly used in downhole applications is also useful herein.

Eroding includes partially or completely removing the metallic layer. Partial removal of the metallic layer during erosion, such as by wearing away patches, strips, or scratches which remove a portion of the surface of the metallic layer and which expose the underlying magnesium alloy, is in some embodiments sufficient to allow penetration of a corrosive material to and dissolution of the magnesium alloy. It will be appreciated that though physical abrasion by proppant is disclosed, the method is not limited to this. Abrasion may also be accomplished by other mechanical means, such as for example by insertion of a downhole tool or element and moving the tool or element with or against the corrodible downhole article to scratch or abrade the metallic layer.

The method further includes corroding the corrodible downhole article in a corrosive material after eroding. The corrosive material includes, for example, water, brine, an acid including hydrochloric acid, hydrogen sulfide, or a combination comprising at least one of the foregoing. In an embodiment, the corrosive material is injected downhole as a slurry containing the proppant, such as for example, a slurry of the proppant in brine, or is injected in a separate operation.

In another embodiment, a method of forming a reversible seal with a corrodible downhole article includes seating a ball or plug in the corrodible downhole article having a shaped surface, such as a concave shape, which accommodates a surface shape such as complementary a convex shape of the ball or plug, the corrodible downhole article comprising a magnesium alloy core, and a metallic layer covering the magnesium alloy core. The metallic layer is resistant to corrosion by a corrosive material as described above. The downhole article prevents fluid flow further downhole when a ball or plug is seated in the downhole article.

Seating is accomplished by placing a ball or plug in the downhole environment, and applying pressure to the downhole environment to effect seating. Placing means, in the case of a ball seat, dropping a ball into the well pipe, and forcing the ball to settle to the ball seat by applying pressure. As discussed above, the balls come in a variety of sizes scaled to seat with specific sized ball seats for isolating different fracture zones. For example, a lower fracture zone has a ball seat accommodating a smaller diameter ball than the ball seat for an upper fracture zone, so that the ball for sealing the lower fracture zone passes through the ball seat for the upper frac-

ture zone, while the ball sized for the upper fracture zone seats on the upper fracture zone ball seat.

Forming the reversible seal further comprises removing the metallic layer of the corrodible downhole article, prior to seating, by injecting a slurry of a proppant into the downhole environment at a pressure greater than that of the downhole environment. During removing, the proppant slurry flows past the article and erodes the metallic layer to expose the magnesium alloy core to the downhole environment. In this way, the ball or plug seats in the corrodible downhole article (e.g., ball seat) directly on the exposed magnesium alloy core.

Unseating of the corrodible downhole article can be accomplished by reducing the pressure applied to the downhole environment. This allows the pressure in the area below the seat to push up the seated ball, when the pressure applied to the downhole environment becomes less than that of the ambient downhole pressure.

In an embodiment, a method of removing a corrodible downhole article includes eroding the metallic layer by physical abrasion, chemical etching, or a combination of physical abrasion and chemical etching as described above, and corroding the corrodible downhole article in a corrosive material after eroding.

Removing the corrodible downhole article is accomplished by corroding the downhole article, after removal of at least a portion of the protective metallic layer, in a corrosive material present downhole. A useful corrosive material includes one of those described herein, and is included with the proppant, or is injected downhole after the proppant. For example, a slurry of a proppant in brine both erodes the metallic layer and corrodes the magnesium alloy core. The abrasive action of the proppant erodes the metallic layer to expose all or a portion of the magnesium alloy core, and the exposed magnesium alloy core then corrodes in the brine of the proppant slurry.

The ball seat 100 is shown in schematic cross-section in FIG. 1. In FIG. 1, a ball seat 100 includes a surface coating layer 111 and magnesium alloy core 112 located in a seating zone 110 for accommodating a ball 130 (with the approximate location of the seated ball 130 shown by dashed lines). The narrowed seating zone 110 is within a housing 120, which is attached to a pipe or tube (not shown). The enclosure 120 has a composition different from that of the magnesium alloy core 112. The ball seat 100, with ball 130 seated in seating zone 110 (after removal of the surface coating layer 111), closes off the lower (narrower) end of the ball seat 100 so that fracking is selectively carried out in the region above the seating zone 110.

In FIG. 2, the process of using the ball seat 200 is shown. In FIG. 2A, the ball seat 200 is shown prior to seating and fracking. A slurry of an abrasive material such as a proppant or other abrasive material is passed into the fracking zone below the ball seat 200 (arrows showing direction of flow) through the seating zone 210, which erodes away all or a portion of the surface coating layer 211 to expose the magnesium alloy core 212. FIG. 2B shows the exposed magnesium alloy core 212, with a ball 230 seated in the seating zone 210 after the surface coating layer 211 has been removed by the action of the proppant. After fracking, the seated ball 230 and the magnesium alloy core 212 are exposed to a corrosive material, such as brine, which dissolves away the magnesium alloy core 212 (and hence seating zone 210). The ball 230 can be removed by dissolving while seated, or can first be unseated. FIG. 2C shows the ball seat 200 after removal (by dissolution) of the seating zone 210, where only housing 220 remains.

While one or more embodiments have been shown and described, modifications and substitutions may be made

thereto without departing from the spirit and scope of the invention. Accordingly, it is to be understood that the present invention has been described by way of illustrations and not limitation.

All ranges disclosed herein are inclusive of the endpoints, and the endpoints are independently combinable with each other. The suffix "(s)" as used herein is intended to include both the singular and the plural of the term that it modifies, thereby including at least one of that term (e.g., the colorant (s) includes at least one colorants). "Optional" or "optionally" means that the subsequently described event or circumstance can or cannot occur, and that the description includes instances where the event occurs and instances where it does not. As used herein, "combination" is inclusive of blends, mixtures, alloys, reaction products, and the like. All references are incorporated herein by reference.

The use of the terms "a" and "an" and "the" and similar referents in the context of describing the invention (especially in the context of the following claims) are to be construed to cover both the singular and the plural, unless otherwise indicated herein or clearly contradicted by context. Further, it should further be noted that the terms "first," "second," and the like herein do not denote any order, quantity, or importance, but rather are used to distinguish one element from another. The modifier "about" used in connection with a quantity is inclusive of the stated value and has the meaning dictated by the context (e.g., it includes the degree of error associated with measurement of the particular quantity).

The invention claimed is:

1. A method of removing a corrodible downhole article having a core and a surface coating disposed on the core, the method comprising:

eroding the surface coating by physical abrasion, chemical etching, or a combination of physical abrasion and chemical etching,

wherein the surface coating comprises:

a metallic layer resistant to corrosion by a corrosive material,

the metallic layer comprising tungsten, cobalt, copper, iron, nickel, aluminum, nickel alloy, aluminum alloy, or a combination comprising at least one of nickel, aluminum, nickel alloy, or aluminum alloy; and

wherein the core comprises magnesium alloy having greater than zero but less than 1 weight percent of nickel.

2. The method of claim 1, wherein the corrodible core comprises magnesium alloy having greater than zero but less than or equal to about 0.5 weight percent of nickel.

3. The method of claim 1, wherein eroding is by physical abrasion alone.

4. The method of claim 1, wherein eroding comprises flowing a slurry of a proppant over the surface coating of the corrodible downhole article.

5. The method of claim 4, wherein the proppant includes sand, aluminum pellets, glass beads, ceramic beads, and combinations comprising at least one of the foregoing.

6. The method of claim 1, further comprising corroding the downhole article in the corrosive material after eroding.

7. The method of claim 6, wherein the corrosive material is water, brine, an acid, hydrogen sulfide, or a combination comprising at least one of the foregoing.

8. The method of claim 1, wherein the metallic layer has a thickness of less than or equal to about 1,000 micrometers.

9. The method of claim 1, wherein the metallic layer is formed by an electroless plating process, or by an electrodeposition process in the presence of an anhydrous ionic solvent.

10. The method of claim 1, wherein the corrodible downhole article is a ball, ball seat or frac plug.

11. The method of claim 1, wherein the metallic layer has a thickness of about 50 to about 750 micrometers.

12. The method of claim 1, wherein the core comprises magnesium alloyed with about 0.25 wt% of Ni.

13. The method of claim 1, wherein the core comprises about 0.25 to about 1 wt% of Ni.

14. A method of forming a reversible seal with a corrodible downhole article, comprising:

seating a ball or plug in the corrodible downhole article having a shaped surface which accommodates a surface shape of the ball or plug, the corrodible downhole article comprising:  
a magnesium alloy core comprising greater than zero but less than or equal to about 1 wt% of nickel, and  
a metallic layer covering the magnesium alloy core, the metallic layer being resistant to corrosion by a corrosive material and comprising tungsten, cobalt, copper, iron, nickel, nickel alloy, aluminum, aluminum alloy, or a combination comprising at least one of nickel, nickel alloy, aluminum, or aluminum alloy;

wherein the corrodible downhole article prevents fluid flow when the ball or plug is seated.

15. The method of claim 14, wherein seating comprises placing the ball or plug in a downhole environment and applying pressure to the downhole environment.

16. The method of claim 15, further comprising removing the metallic layer of the corrodible downhole article, prior to seating, by injecting a slurry of a proppant into the downhole environment at a pressure greater than that of the downhole environment.

17. The method of claim 16, wherein the proppant slurry flows past the article and erodes the metallic layer to expose the magnesium alloy core.

18. The method of claim 17, further comprising corroding the exposed magnesium alloy core in a corrosive material.

19. The method of claim 15, further comprising unseating the ball or the plug seated in the corrodible downhole article by reducing the pressure applied to the downhole environment to a pressure below that of an ambient downhole pressure.

20. A method of removing a corrodible downhole article comprising:

a core, and  
a metallic layer covering the core,  
the method comprising eroding the metallic layer by physical abrasion, chemical etching, or a combination of physical abrasion and chemical etching, and  
corroding the corrodible downhole article in a corrosive material after eroding,

wherein the core of the corrodible downhole article comprises magnesium alloy and greater than zero but less than or equal to about 1 wt% of nickel; and

the metallic layer of the downhole article comprises tungsten, cobalt, copper, iron, nickel, nickel alloy, aluminum, aluminum alloy, or a combination comprising at least one of nickel, nickel alloy, aluminum, or aluminum alloy.